



US007244540B2

(12) **United States Patent**  
**Zhu et al.**

(10) **Patent No.:** **US 7,244,540 B2**  
(45) **Date of Patent:** **Jul. 17, 2007**

(54) **LIQUID TONERS COMPRISING  
AMPHIPATHIC COPOLYMERIC BINDER  
HAVING INSOLUBLE COMPONENTS IN  
THE SHELL PORTION THEREOF**

(75) Inventors: **Jiayi Zhu**, Woodbury, MN (US); **Gay L. Herman**, Cottage Grove, MN (US)

(73) Assignee: **Samsung Electronics Company**, Suwon (KR)

(\*) Notice: Subject to any disclaimer, the term of this patent is extended or adjusted under 35 U.S.C. 154(b) by 430 days.

(21) Appl. No.: **10/975,557**

(22) Filed: **Oct. 28, 2004**

(65) **Prior Publication Data**

US 2006/0093949 A1 May 4, 2006

(51) **Int. Cl.**  
**G03G 9/13** (2006.01)

(52) **U.S. Cl.** ..... 430/114; 430/137.22

(58) **Field of Classification Search** ..... 430/114,  
430/115

See application file for complete search history.

(56) **References Cited**

U.S. PATENT DOCUMENTS

|             |         |                        |            |
|-------------|---------|------------------------|------------|
| 4,157,974 A | 6/1979  | Brechlin et al. ....   | 430/137.19 |
| 4,413,048 A | 11/1983 | Landa .....            | 430/115    |
| 4,473,629 A | 9/1984  | Herrmann et al. ....   | 430/114    |
| 4,497,886 A | 2/1985  | Herrmann et al. ....   | 430/115    |
| 4,594,305 A | 6/1986  | Vollmann et al. ....   | 430/115    |
| 4,925,766 A | 5/1990  | Elmasry et al. ....    | 430/115    |
| 4,946,753 A | 8/1990  | Elmasry et al. ....    | 430/45     |
| 4,978,598 A | 12/1990 | Elmasry et al. ....    | 430/137.17 |
| 4,988,602 A | 1/1991  | Jongewaard et al. .... | 430/115    |
| 5,061,583 A | 10/1991 | Zwadlo et al. ....     | 430/45     |
| 5,066,559 A | 11/1991 | Elmasry et al. ....    | 430/115    |

|             |         |                        |            |
|-------------|---------|------------------------|------------|
| 5,089,362 A | 2/1992  | Chou et al. ....       | 430/16     |
| 5,302,482 A | 4/1994  | Elmasry et al. ....    | 430/115    |
| 5,322,751 A | 6/1994  | Chou et al. ....       | 430/33     |
| 5,557,311 A | 9/1996  | Perrington et al. .... | 347/111    |
| 5,604,070 A | 2/1997  | Rao et al. ....        | 430/108.22 |
| 5,650,253 A | 7/1997  | Baker et al. ....      | 430/119    |
| 5,652,282 A | 7/1997  | Baker et al. ....      | 523/201    |
| 5,698,616 A | 12/1997 | Baker et al. ....      | 523/201    |
| 5,753,763 A | 5/1998  | Rao et al. ....        | 525/276    |
| 5,886,067 A | 3/1999  | Li et al. ....         | 523/201    |
| 5,893,658 A | 4/1999  | Kellie et al. ....     | 399/40     |

(Continued)

OTHER PUBLICATIONS

Commonly assigned U.S. Appl. No. 10/975,526, filed Oct. 28, 2004 entitled "Dry Toners Comprising Amphipathic Copolymeric Binder Having Non-Sorptive Components in the Shell Portion Thereof", in the Name of Jiayi Zhu et al.

Primary Examiner—Barbara L. Gilliam

Assistant Examiner—Rachel Burney

(74) Attorney, Agent, or Firm—Kagan Binder, PLLC

(57) **ABSTRACT**

The invention provides liquid electrographic toner compositions comprising a liquid carrier having toner particles dispersed in the liquid carrier. The liquid carrier has a Kauri-Butanol number less than about 30 mL. The toner particles comprise polymeric binder comprising at least one amphipathic copolymer comprising one or more S material portions and one or more D material portions. The S material portion comprises at least one soluble component and at least one insoluble component, wherein the insoluble component is the reaction product of monomers having an absolute difference in Hildebrand solubility parameter from the liquid carrier of about 3.0 MPa<sup>1/2</sup> or greater. These toner particles can exhibit excellent final image durability characteristics, and can also provide toner compositions that provide excellent images at low fusion temperatures on a final image receptor.

19 Claims, 3 Drawing Sheets



U.S. PATENT DOCUMENTS

|             |         |                    |         |                 |         |                      |           |
|-------------|---------|--------------------|---------|-----------------|---------|----------------------|-----------|
| 5,916,718 A | 6/1999  | Kellie et al. .... | 430/45  | 6,171,740 B1    | 1/2001  | Fonash et al. ....   | 430/52    |
| 5,919,866 A | 7/1999  | Rao et al. ....    | 525/276 | 6,255,363 B1    | 7/2001  | Baker et al. ....    | 523/201   |
| 5,970,273 A | 10/1999 | Zenk et al. ....   | 399/12  | 6,357,351 B1    | 3/2002  | Bhambra et al. ....  | 101/455   |
| 5,991,588 A | 11/1999 | Kraft ....         | 399/297 | 6,391,912 B1    | 5/2002  | Hagemann et al. .... | 504/116.1 |
| 6,088,560 A | 7/2000  | Zenk et al. ....   | 399/237 | 6,633,735 B2    | 10/2003 | Kellie et al. ....   | 399/55    |
| 6,103,781 A | 8/2000  | Li et al. ....     | 523/201 | 2004/0091807 A1 | 5/2004  | Qian et al. ....     | 430/114   |
|             |         |                    |         | 2004/0091809 A1 | 5/2004  | Qian et al. ....     | 430/114   |

**Figure 1**

**Figure 2**

**Figure 3**

**LIQUID TONERS COMPRISING  
AMPHIPATHIC COPOLYMERIC BINDER  
HAVING INSOLUBLE COMPONENTS IN  
THE SHELL PORTION THEREOF**

**FIELD OF THE INVENTION**

The present invention relates to liquid toner compositions having utility in electrography. More particularly, the invention relates to liquid toner compositions comprising an amphipathic copolymer binder having an insoluble component in the shell portion of the copolymer.

**BACKGROUND OF THE INVENTION**

In electrophotographic and electrostatic printing processes (collectively electrographic processes), an electrostatic image is formed on the surface of a photoreceptive element or dielectric element, respectively. The photoreceptive element or dielectric element can be an intermediate transfer drum or belt or the substrate for the final toned image itself, as described by Schmidt, S. P. and Larson, J. R. in *Handbook of Imaging Materials* Diamond, A. S., Ed: Marcel Dekker: New York; Chapter 6, pp 227-252, and U.S. Pat. Nos. 4,728,983, 4,321,404, and 4,268,598.

Electrophotography forms the technical basis for various well-known imaging processes, including photocopying and some forms of laser printing. Other imaging processes use electrostatic or ionographic printing. Electrostatic printing is printing where a dielectric receptor or substrate is "written" upon imagewise by a charged stylus, leaving a latent electrostatic image on the surface of the dielectric receptor. This dielectric receptor is not photosensitive and is generally not re-useable. Once the image pattern has been "written" onto the dielectric receptor in the form of an electrostatic charge pattern of positive or negative polarity, oppositely charged toner particles are applied to the dielectric receptor in order to develop the latent image. An exemplary electrostatic imaging process is described in U.S. Pat. No. 5,176,974.

In contrast, electrophotographic imaging processes typically involve the use of a reusable, light sensitive, temporary image receptor, known as a photoreceptor, in the process of producing an electrophotographic image on a final, permanent image receptor. A representative electrophotographic process involves a series of steps to produce an image on a receptor, including charging, exposure, development, transfer, fusing, cleaning, and erasure.

In the charging step, a photoreceptor is covered with charge of a desired polarity, either negative or positive, typically with a corona or charging roller. In the exposure step, an optical system, typically a laser scanner or diode array, forms a latent image by selectively exposing the photoreceptor to electromagnetic radiation, thereby discharging the charged surface of the photoreceptor in an imagewise manner corresponding to the desired image to be formed on the final image receptor. The electromagnetic radiation, which can also be referred to as "light," can include infrared radiation, visible light, and ultraviolet radiation, for example.

In the development step, toner particles of the appropriate polarity are generally brought into contact with the latent image on the photoreceptor, typically using a developer electrically-biased to a potential having the same polarity as the toner polarity. The toner particles migrate to the photoreceptor and selectively adhere to the latent image via electrostatic forces, forming a toned image on the photoreceptor.

In the transfer step, the toned image is transferred from the photoreceptor to the desired final image receptor; an intermediate transfer element is sometimes used to effect transfer of the toned image from the photoreceptor with subsequent transfer of the toned image to a final image receptor. The transfer of an image typically occurs by one of the following two methods: elastomeric assist (also referred to herein as "adhesive transfer") or electrostatic assist (also referred to herein as "electrostatic transfer").

10 Elastomeric assist or adhesive transfer refers generally to a process in which the transfer of an image is primarily caused by balancing the relative energies between the ink, a photoreceptor surface and a temporary carrier surface or medium for the toner. The effectiveness of such elastomeric assist or adhesive transfer is controlled by several variables including surface energy, temperature, pressure, and toner rheology. An exemplary elastomeric assist/adhesive image transfer process is described in U.S. Pat. No. 5,916,718.

15 Electrostatic assist or electrostatic transfer refers generally to a process in which transfer of an image is primarily affected by electrostatic charges or charge differential phenomena between the receptor surface and the temporary carrier surface or medium for the toner. Electrostatic transfer can be influenced by surface energy, temperature, and pressure, but the primary driving forces causing the toner image to be transferred to the final substrate are electrostatic forces. An exemplary electrostatic transfer process is described in U.S. Pat. No. 4,420,244.

20 In the fusing step, the toned image on the final image receptor is heated to soften or melt the toner particles, thereby fusing the toned image to the final receptor. An alternative fusing method involves fixing the toner to the final receptor under high pressure with or without heat. In the cleaning step, residual toner remaining on the photoreceptor is removed. Finally, in the erasing step, the photoreceptor charge is reduced to a substantially uniformly low value by exposure to light of a particular wavelength band, thereby removing remnants of the original latent image and preparing the photoreceptor for the next imaging cycle.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 986

Two types of toner are in widespread, commercial use: liquid toner and dry toner. The term "dry" does not mean that the dry toner is totally free of any liquid constituents, but connotes that the toner particles do not contain any significant amount of solvent, e.g., typically less than 10 weight percent solvent (generally, dry toner is as dry as is reasonably practical in terms of solvent content), and are capable of carrying a triboelectric charge. This distinguishes dry toner particles from liquid toner particles.

A typical liquid toner composition generally includes toner particles suspended or dispersed in a liquid carrier. The liquid carrier is typically a nonconductive dispersant, to avoid discharging the latent electrostatic image. Liquid toner particles are generally solvated to some degree in the liquid carrier (or carrier liquid), typically in more than 50 weight percent of a low polarity, low dielectric constant, substantially nonaqueous carrier solvent. Liquid toner particles are generally chemically charged using polar groups that dissociate in the carrier solvent, but do not carry a triboelectric charge while solvated and/or dispersed in the liquid carrier. Liquid toner particles are also typically smaller than dry toner particles. Because of their small particle size, ranging from about 5 microns to sub-micron, liquid toners are capable of producing very high-resolution toned images, and are therefore preferred for high resolution, multi-color printing applications.

A typical toner particle for a liquid toner composition generally comprises a visual enhancement additive (for example, a colored pigment particle) and a polymeric binder. The polymeric binder fulfills functions both during and after the electrographic process. With respect to processability, the character of the binder impacts charging and charge stability, flow, and fusing characteristics of the toner particles. These characteristics are important to achieve good performance during development, transfer, and fusing. After an image is formed on the final receptor, the nature of the binder (e.g. glass transition temperature, melt viscosity, molecular weight) and the fusing conditions (e.g. temperature, pressure and fuser configuration) impact durability (e.g. blocking and erasure resistance), adhesion to the receptor, gloss, and the like. Exemplary liquid toners and liquid electrophotographic imaging process are described by Schmidt, S. P. and Larson, J. R. in *Handbook of Imaging Materials* Diamond, A. S., Ed: Marcel Dekker: New York; Chapter 6, pp 227-252.

The liquid toner composition can vary greatly with the type of transfer used because liquid toner particles used in adhesive transfer imaging processes must be "film-formed" and have adhesive properties after development on the photoreceptor, while liquid toners used in electrostatic transfer imaging processes must remain as distinct charged particles after development on the photoreceptor.

Toner particles useful in adhesive transfer processes generally have effective glass transition temperatures below approximately 30° C. and volume mean particle diameter between 0.1-1 micron. In addition, for liquid toners used in adhesive transfer imaging processes, the carrier liquid generally has a vapor pressure sufficiently high to ensure rapid evaporation of solvent following deposition of the toner onto a photoreceptor, transfer belt, and/or receptor sheet. This is particularly true for cases in which multiple colors are sequentially deposited and overlaid to form a single image, because in adhesive transfer systems, the transfer is promoted by a drier toned image that has high cohesive strength (commonly referred to as being "film formed"). Generally, the toned imaged should be dried to higher than approximately 68-74 volume percent solids in order to be "film-

formed" sufficiently to exhibit good adhesive transfer. U.S. Pat. No. 6,255,363 describes the formulation of liquid electrophotographic toners suitable for use in imaging processes using adhesive transfer.

In contrast, toner particles useful in electrostatic transfer processes generally have effective glass transition temperatures above approximately 40° C. and volume mean particle diameter between 3-10 microns. For liquid toners used in electrostatic transfer imaging processes, the toned image is preferably no more than approximately 30% w/w solids for good transfer. A rapidly evaporating carrier liquid is therefore not preferred for imaging processes using electrostatic transfer. U.S. Pat. No. 4,413,048 describes the formulation of one type of liquid electrophotographic toner suitable for use in imaging processes using electrostatic transfer.

The art continually searches for improved liquid toner compositions that produce high quality, durable images at low fusion temperatures on a final image receptor.

## SUMMARY OF THE INVENTION

The present invention relates to liquid electrographic toner compositions comprising a liquid carrier having toner particles dispersed in the liquid carrier. The liquid carrier has a Kauri-Butanol number less than about 30 mL. The toner particles comprise polymeric binder comprising at least one amphiphilic copolymer comprising one or more S material portions and one or more D material portions.

In prior amphiphilic copolymer systems, the S material portion has been carefully selected to assure that the resulting toner particle would be readily dispersed in the liquid carrier. To achieve this effect, the S material portion has been prepared from monomeric materials that are soluble in the liquid carrier. The present invention, in contrast, provides amphiphilic copolymers wherein the S material portion comprises at least one soluble component and at least one insoluble component. This insoluble component is the reaction product of monomers having an absolute difference in Hildebrand solubility parameter from the liquid carrier of about 3.0 MPa<sup>1/2</sup> or greater. Preferably, the insoluble component is the reaction product of monomers having an absolute difference in Hildebrand solubility parameter from the liquid carrier of about 3.15 MPa<sup>1/2</sup> or greater, more preferably of about 3.30 MPa<sup>1/2</sup> or greater or of about 3.40 MPa<sup>1/2</sup> or greater.

Surprisingly, this formulation of amphiphilic copolymer provides toners that can exhibit excellent final image durability characteristics, and can also provide a toner composition that provides excellent images at low fusion temperatures on a final image receptor. The images that are formed from toner compositions of the present invention can exhibit excellent durability and erasure resistance properties.

## BRIEF DESCRIPTION OF THE DRAWINGS

FIG. 1 is a graph showing the fused image erasure resistances vs. fusing temperatures for various toner formulations.

FIG. 2 is a graph showing the fused image erasure resistances vs. fusing temperatures for additional toner formulations.

FIG. 3 is a graph showing the fused image erasure resistances vs. fusing temperatures for additional toner formulations.

DETAILED DESCRIPTION OF PRESENTLY  
PREFERRED EMBODIMENTS

The embodiments of the present invention described below are not intended to be exhaustive or to limit the invention to the precise forms disclosed in the following detailed description. Rather, the embodiments are chosen and described so that others skilled in the art can appreciate and understand the principles and practices of the present invention.

The toner particles of the liquid toner composition comprise a polymeric binder that comprises an amphiphilic copolymer. The term "amphiphilic" refers to a copolymer having a combination of portions having distinct solubility and dispersibility characteristics in a desired liquid carrier that is used to make the organosol and/or used in the course of preparing the liquid toner particles. Preferably, the liquid carrier is selected such that at least one portion (also referred to herein as S material or portion(s)) of the copolymer is more solvated by the carrier while at least one other portion (also referred to herein as D material or portion(s)) of the copolymer constitutes more of a dispersed phase in the carrier.

Preferably, the nonaqueous liquid carrier of the organosol is selected such that at least one portion (also referred to herein as the S material or portion) of the amphiphilic copolymer is more solvated by the carrier while at least one other portion (also referred to herein as the D material or portion) of the copolymer constitutes more of a dispersed phase in the carrier. In other words, preferred copolymers of the present invention comprise S and D material having respective solubilities in the desired liquid carrier that are sufficiently different from each other such that the S blocks tend to be more solvated by the carrier while the D blocks tend to be more dispersed in the carrier. More preferably, the S blocks are soluble in the liquid carrier while the D blocks are insoluble. In particularly preferred embodiments, the D material phase separates from the liquid carrier, forming dispersed particles.

From one perspective, the polymer particles when dispersed in the liquid carrier can be viewed as having a core/shell structure in which the D material tends to be in the core, while the S material tends to be in the shell. The S material thus functions as a dispersing aid, steric stabilizer or graft copolymer stabilizer, to help stabilize dispersions of the copolymer particles in the liquid carrier. Consequently, the S material can also be referred to herein as a "graft stabilizer." The core/shell structure of the binder particles tends to be retained when the particles are dried when incorporated into liquid toner particles.

The solubility of a material, or a portion of a material such as a copolymeric portion, can be qualitatively and quantitatively characterized in terms of its Hildebrand solubility parameter. The Hildebrand solubility parameter refers to a solubility parameter represented by the square root of the cohesive energy density of a material, having units of  $(\text{pressure})^{1/2}$ , and being equal to  $(\Delta H/RT)^{1/2}/V^{1/2}$ , where  $\Delta H$  is the molar vaporization enthalpy of the material,  $R$  is the universal gas constant,  $T$  is the absolute temperature, and  $V$  is the molar volume of the solvent. Hildebrand solubility parameters are tabulated for solvents in Barton, A. F. M., *Handbook of Solubility and Other Cohesion Parameters*, 2d Ed. CRC Press, Boca Raton, Fla., (1991), for monomers and representative polymers in *Polymer Handbook*, 3rd Ed., J. Brandrup & E. H. Immergut, Eds. John Wiley, N.Y., pp 519-557 (1989), and for many commercially available polymers in Barton, A. F. M., *Handbook of Polymer-Liquid*

Interaction Parameters and Solubility Parameters, CRC  
Press, Boca Raton, Fla., (1990).

The degree of solubility of a material, or portion thereof, in a liquid carrier can be predicted from the absolute difference in Hildebrand solubility parameters between the material, or portion thereof, and the liquid carrier. A material, or portion thereof, will be fully soluble or at least in a highly solvated state when the absolute difference in Hildebrand solubility parameter between the material, or portion thereof, and the liquid carrier is less than approximately  $1.5 \text{ MPa}^{1/2}$ . On the other hand, when the absolute difference between the Hildebrand solubility parameters exceeds approximately  $3.0 \text{ MPa}^{1/2}$ , the material, or portion thereof, will tend to phase separate from the liquid carrier, forming a dispersion. When the absolute difference in Hildebrand solubility parameters is between  $1.5 \text{ MPa}^{1/2}$  and  $3.0 \text{ MPa}^{1/2}$ , the material, or portion thereof, is considered to be weakly solvatable or marginally insoluble in the liquid carrier.

Consequently, in preferred embodiments, the absolute difference between the respective Hildebrand solubility parameters of the S material portion(s) of the copolymer and the liquid carrier is less than  $3.0 \text{ MPa}^{1/2}$ . In a preferred embodiment of the present invention, the absolute difference between the respective Hildebrand solubility parameters of the S material portion(s) of the copolymer and the liquid carrier is from about 2 to about  $3.0 \text{ MPa}^{1/2}$ . In a particularly preferred embodiment of the present invention, the absolute difference between the respective Hildebrand solubility parameters of the S material portion(s) of the copolymer and the liquid carrier is from about 2.5 to about  $3.0 \text{ MPa}^{1/2}$ . Additionally, it is also preferred that the absolute difference between the respective Hildebrand solubility parameters of the D material portion(s) of the copolymer and the liquid carrier is greater than  $2.3 \text{ MPa}^{1/2}$ , preferably greater than about  $2.5 \text{ MPa}^{1/2}$ , more preferably greater than about  $3.0 \text{ MPa}^{1/2}$ , with the proviso that the difference between the respective Hildebrand solubility parameters of the S and D material portion(s) is at least about  $0.4 \text{ MPa}^{1/2}$ , more preferably at least about  $1.0 \text{ MPa}^{1/2}$ . Because the Hildebrand solubility of a material can vary with changes in temperature, such solubility parameters are preferably determined at a desired reference temperature such as at  $25^\circ \text{C}$ .

As noted above, the S material portion comprises an insoluble component that is the reaction product of monomers having an absolute difference in Hildebrand solubility parameter from the liquid carrier of about  $3.0 \text{ MPa}^{1/2}$  or greater. The S material portion, notwithstanding the presence of the insoluble component, must have an overall solubility characteristic to be soluble in the carrier liquid. Thus, the S material portion as a whole preferably meets the specified and preferred ranges of solubility parameter as discussed above, notwithstanding the presence of the insoluble component. The S material portion may be prepared by incorporation of a single type of monomer that exhibits the desired solubility parameter as the insoluble component, or may be prepared by incorporation of a plurality of monomers, each of which exhibits the desired solubility parameter as the insoluble component. In a preferred embodiment of the present invention, the insoluble component is present in an amount of from about 1% to about 40% of the S material portion (not counting the anchoring group functionality if present in the graft copolymer). In another preferred embodiment, the insoluble component is present in an amount of from about 1% to about 20% or from about 1% to about 5% of the S material portion

Those skilled in the art understand that the Hildebrand solubility parameter for a copolymer, or portion thereof, can

be calculated using a volume fraction weighting of the individual Hildebrand solubility parameters for each monomer comprising the copolymer, or portion thereof, as described for binary copolymers in Barton A. F. M., *Handbook of Solubility Parameters and Other Cohesion Parameters*, CRC Press, Boca Raton, p 12 (1990). The magnitude of the Hildebrand solubility parameter for polymeric materials is also known to be weakly dependent upon the weight average molecular weight of the polymer, as noted in Barton, pp 446–448. Thus, there will be a preferred molecular weight range for a given polymer or portion thereof in order to achieve desired solvating or dispersing characteristics. Similarly, the Hildebrand solubility parameter for a mixture can be calculated using a volume fraction weighting of the individual Hildebrand solubility parameters for each component of the mixture.

In addition, we have defined our invention in terms of the calculated solubility parameters of the monomers and solvents obtained using the group contribution method developed by Small, P. A., *J. Appl. Chem.*, 3, 71 (1953) using Small's group contribution values listed in Table 2.2 on page VII/525 in the Polymer Handbook, 3rd Ed., J. Brandrup & E. H. Immergut, Eds. John Wiley, New York, (1989). We have chosen this method for defining our invention to avoid ambiguities which could result from using solubility parameter values obtained with different experimental methods. In addition, Small's group contribution values will generate solubility parameters that are consistent with data derived from measurements of the enthalpy of vaporization, and therefore are completely consistent with the defining expression for the Hildebrand solubility parameter. Since it is not practical to measure the heat of vaporization for polymers, monomers are a reasonable substitution.

For purposes of illustration, Table I lists Hildebrand solubility parameters for some common solvents used in an electrographic toner and the Hildebrand solubility parameters and glass transition temperatures (based on their high molecular weight homopolymers) for some common monomers used in synthesizing organosols.

TABLE I

| Hildebrand Solubility Parameters |                                                    |                                                       |
|----------------------------------|----------------------------------------------------|-------------------------------------------------------|
| Solvent Values at 25° C.         |                                                    |                                                       |
| Solvent Name                     | Kauri-Butanol Number by ASTM Method D1133-54T (ml) | Hildebrand Solubility Parameter (MPa <sup>1/2</sup> ) |
| Norpar™ 15                       | 18                                                 | 13.99                                                 |
| Norpar™ 13                       | 22                                                 | 14.24                                                 |
| Norpar™ 12                       | 23                                                 | 14.30                                                 |
| Isopar™ V                        | 25                                                 | 14.42                                                 |
| Isopar™ G                        | 28                                                 | 14.60                                                 |
| Exxsol™ D80                      | 28                                                 | 14.60                                                 |

Source: Calculated from equation #31 of Polymer Handbook, 3rd Ed., J. Brandrup E. H. Immergut, Eds. John Wiley, NY, p. VII/522 (1989).

Monomer Values at 25° C.

| Monomer Name                            | Hildebrand Solubility Parameter (MPa <sup>1/2</sup> ) | Glass Transition Temperature (° C.)* |
|-----------------------------------------|-------------------------------------------------------|--------------------------------------|
| 3,3,5-Trimethyl Cyclohexyl Methacrylate | 16.73                                                 | 125                                  |
| Isobornyl Methacrylate                  | 16.90                                                 | 110                                  |
| Isobornyl Acrylate                      | 16.01                                                 | 94                                   |
| n-Behenyl acrylate                      | 16.74                                                 | <-55 (58 m.p.)*                      |

TABLE I-continued

| Hildebrand Solubility Parameters |                           |       |
|----------------------------------|---------------------------|-------|
| 5                                | n-Octadecyl Methacrylate  | 16.77 |
|                                  | n-Octadecyl Acrylate      | 16.82 |
|                                  | Lauryl Methacrylate       | 16.84 |
|                                  | Lauryl Acrylate           | 16.95 |
|                                  | 2-Ethylhexyl Methacrylate | 16.97 |
|                                  | 2-Ethylhexyl Acrylate     | 17.03 |
| 10                               | n-Hexyl Methacrylate      | 17.13 |
|                                  | t-Butyl Methacrylate      | 17.16 |
|                                  | n-Butyl Methacrylate      | 17.22 |
|                                  | n-Hexyl Acrylate          | 17.30 |
|                                  | n-Butyl Acrylate          | 17.45 |
|                                  | Ethyl Methacrylate        | 17.62 |
| 15                               | Ethyl Acrylate            | 18.04 |
|                                  | Methyl Methacrylate       | 18.17 |
|                                  | Styrene                   | 18.05 |

Calculated using Small's Group Contribution Method, Small, P. A. *Journal of Applied Chemistry* 3 p. 71 (1953). Using Group Contributions from Polymer Handbook, 3rd Ed., J. Brandrup E. H. Immergut, Eds., John Wiley, NY, p. VII/525 (1989).

\*Polymer Handbook, 3rd Ed., J. Brandrup E. H. Immergut, Eds., John Wiley, NY, pp. VII/209–277 (1989). The  $T_g$  listed is for the homopolymer of the respective monomer.

\*\*m.p. refers to melting point for selected Polymerizable Crystallizable Compounds.

25 The liquid carrier is a substantially nonaqueous solvent or solvent blend. In other words, only a minor component (generally less than 25 weight percent) of the liquid carrier comprises water. Preferably, the substantially nonaqueous liquid carrier comprises less than 20 weight percent water, more preferably less than 10 weight percent water, even more preferably less than 3 weight percent water, most preferably less than one weight percent water.

30 The substantially nonaqueous liquid carrier can be selected from a wide variety of materials, or combination of materials, which are known in the art, but preferably has a Kauri-butanol number less than 30 ml. The liquid is preferably oleophilic, chemically stable under a variety of conditions, and electrically insulating. Electrically insulating refers to a dispersant liquid having a low dielectric constant and a high electrical resistivity. Preferably, the liquid dispersant has a dielectric constant of less than 5; more preferably less than 3. Electrical resistivities of carrier liquids are typically greater than  $10^9$  Ohm-cm; more preferably greater than  $10^{10}$  Ohm-cm. In addition, the liquid carrier desirably is chemically inert in most embodiments with respect to the ingredients used to formulate the toner particles.

35 Examples of suitable liquid carriers include aliphatic hydrocarbons (n-pentane, hexane, heptane and the like), cycloaliphatic hydrocarbons (cyclopentane, cyclohexane and the like), aromatic hydrocarbons (benzene, toluene, xylene and the like), halogenated hydrocarbon solvents (chlorinated alkanes, fluorinated alkanes, chlorofluorocarbons and the like) silicone oils and blends of these solvents.

40 Preferred liquid carriers include branched paraffinic solvent blends such as Isopar™G, Isopar™H, Isopar™K, Isopar™L, Isopar™M and Isopar™V (available from Exxon Corporation, NJ), and most preferred carriers are the aliphatic hydrocarbon solvent blends such as Norpar™12, Norpar™13 and Norpar™15 (available from Exxon Corporation, NJ). Particularly preferred liquid carriers have a Hildebrand solubility parameter of from about 13 to about 15 MPa<sup>1/2</sup>.

45 55 The liquid carrier of the toner compositions of the present invention is preferably the same liquid as used as the solvent for preparation of the amphipathic copolymer. Alternatively,

the polymerization can be carried out in any appropriate solvent, and a solvent exchange can be carried out to provide the desired liquid carrier for the toner composition.

As used herein, the term "copolymer" encompasses both oligomeric and polymeric materials, and encompasses polymers incorporating two or more monomers. As used herein, the term "monomer" means a relatively low molecular weight material (i.e., generally having a molecular weight less than about 500 Daltons) having one or more polymerizable groups. "Oligomer" means a relatively intermediate sized molecule incorporating two or more monomers and generally having a molecular weight of from about 500 up to about 10,000 Daltons. "Polymer" means a relatively large material comprising a substructure formed two or more monomeric, oligomeric, and/or polymeric constituents and generally having a molecular weight greater than about 10,000 Daltons.

The weight average molecular weight of the amphiphatic copolymer of the present invention can vary over a wide range, and can impact imaging performance. The polydispersity of the copolymer also can impact imaging and transfer performance of the resultant liquid toner material. Because of the difficulty of measuring molecular weight for an amphiphatic copolymer, the particle size of the dispersed copolymer (organosol) can instead be correlated to imaging and transfer performance of the resultant liquid toner material. Generally, the volume mean particle diameter ( $D_v$ ) of the dispersed graft copolymer particles, determined by laser diffraction particle size measurement, should be in the range 1–100 microns, more preferably 5–75 microns, and most preferably 10–50 microns.

In addition, a correlation exists between the molecular weight of the solvatable or soluble S material portion of the graft copolymer, and the imaging and transfer performance of the resultant toner. Generally, the S material portion of the copolymer has a weight average molecular weight in the range of 1000 to about 1,000,000 Daltons, preferably 5000 to 400,000 Daltons, more preferably 50,000 to 300,000 Daltons. It is also generally desirable to maintain the polydispersity (the ratio of the weight-average molecular weight to the number average molecular weight) of the S material portion of the copolymer below 15, more preferably below 5, most preferably below 2.5. It is a distinct advantage of the present invention that copolymer particles with such lower polydispersity characteristics for the S material portion are easily made in accordance with the practices described herein, particularly those embodiments in which the copolymer is formed in the liquid carrier *in situ*.

The relative amounts of S and D material portions in a copolymer can impact the solvating and dispersability characteristics of these portions. For instance, if too little of the S material portion(s) are present, the copolymer can have too little stabilizing effect to sterically stabilize the organosol with respect to aggregation as might be desired. If too little of the D material portion(s) are present, the small amount of D material can be too soluble in the liquid carrier such that there can be insufficient driving force to form a distinct particulate, dispersed phase in the liquid carrier. The presence of both a solvated and dispersed phase helps the ingredients of particles self assemble *in situ* with exceptional uniformity among separate particles. Balancing these concerns, the preferred weight ratio of D material to S material is in the range of 1/20 to 20/1, preferably 1/1 to 15/1, more preferably 2/1 to 10/1, and most preferably 4/1 to 8/1.

Glass transition temperature,  $T_g$ , refers to the temperature at which a (co)polymer, or portion thereof, changes from a hard, glassy material to a rubbery, or viscous, material,

corresponding to a dramatic increase in free volume as the (co)polymer is heated. The  $T_g$  can be calculated for a (co)polymer, or portion thereof, using known  $T_g$  values for the high molecular weight homopolymers (see, e.g., Table I herein) and the Fox equation expressed below:

$$1/T_g = w_1/T_{g1} + w_2/T_{g2} + \dots + w_i/T_{gi}$$

wherein each  $w_n$  is the weight fraction of monomer "n" and each  $T_{gn}$  is the absolute glass transition temperature (in degrees Kelvin) of the high molecular weight homopolymer of monomer "n" as described in Wicks, A. W., F. N. Jones & S. P. Pappas, *Organic Coatings 1*, John Wiley, NY, pp 54–55 (1992).

In the practice of the present invention, values of  $T_g$  for the D or S material portion of the copolymer or of the soluble polymer were determined either using the Fox equation above or experimentally, using e.g., differential scanning calorimetry. The glass transition temperatures ( $T_g$ 's) of the S and D material portions can vary over a wide range and can be independently selected to enhance manufacturability and/or performance of the resulting liquid toner particles. The  $T_g$ 's of the S and D material portions will depend to a large degree upon the type of monomers constituting such portions. Consequently, to provide a copolymer material with higher  $T_g$ , one can select one or more higher  $T_g$  monomers with the appropriate solubility characteristics for the type of copolymer portion (D or S) in which the monomer(s) will be used. Conversely, to provide a copolymer material with lower  $T_g$ , one can select one or more lower  $T_g$  monomers with the appropriate solubility characteristics for the type of portion in which the monomer(s) will be used.

For copolymers useful in liquid toner applications, the copolymer  $T_g$  preferably should not be too low or else receptors printed with the toner can experience undue blocking. Conversely, the minimum fusing temperature required to soften or melt the toner particles sufficient for them to adhere to the final image receptor will increase as the copolymer  $T_g$  increases. Consequently, it is preferred that the  $T_g$  of the copolymer be far enough above the expected maximum storage temperature of a printed receptor so as to avoid blocking issues, yet not so high as to require fusing temperatures approaching the temperatures at which the final image receptor can be damaged, e.g. approaching the autoignition temperature of paper used as the final image receptor. Desirably, therefore, the copolymer has a  $T_g$  of 30–125° C., more preferably 40–100° C., most preferably 50–80° C. For copolymers in which the D material portion comprises a major portion of the copolymer, the  $T_g$  of the D material portion will dominate the  $T_g$  of the copolymer as a whole. In one embodiment of copolymers useful in liquid toner applications, it is preferred that the  $T_g$  of the D material portion fall in the range of 30–105° C., more preferably 40–85° C., most preferably 60–75° C., since the S material portion will generally exhibit a lower  $T_g$  than the D material portion, and a higher  $T_g$  D material portion is therefore desirable to offset the  $T_g$  lowering effect of the S material portion, which can be solvatable. Blocking with respect to the S material portion material is not as significant an issue inasmuch as preferred copolymers comprise a majority of the D material portion material. Consequently, the  $T_g$  of the D material portion material will dominate the effective  $T_g$  of the copolymer as a whole. However, if the  $T_g$  of the S material portion is too low, then the particles might tend to aggregate. On the other hand, if the  $T_g$  is too high, then the requisite fusing temperature can be too high. Balancing

## 11

these concerns, the S material portion material in one embodiment is preferably formulated to have a  $T_g$  of at least 0° C., preferably at least 20° C., more preferably at least 40° C. Surprisingly, it has been discovered that by providing amphiphatic copolymers wherein the S material portion comprises at least one soluble component and at least one insoluble component, the S material portion may have a measured  $T_g$  that is considerably lower than conventional  $T_g$ 's, while still being effective as liquid toner compositions. Thus, in one embodiment the S material portion material is preferably formulated to have a  $T_g$  of from about -40° C. to 20° C. It is understood that the requirements imposed on the self-fixing characteristics of a liquid toner will depend to a great extent upon the nature of the imaging process. For example, rapid self-fixing of the toner to form a cohesive film may not be required or even desired in an electrographic imaging process if the image is not subsequently transferred to a final receptor, or if the transfer is effected by means (e.g. electrostatic transfer) not requiring a film formed toner on a temporary image receptor (e.g. a photoreceptor).

Similarly, in multi-color (or multi-pass) electrostatic printing wherein a stylus is used to generate a latent electrostatic image directly upon a dielectric receptor that serves as the final toner receptor material, a rapidly self-fixing toner film can be undesirably removed in passing under the stylus. This head scraping can be reduced or eliminated by manipulating the effective glass transition temperature of the organosol. For liquid electrographic (electrostatic) toners, particularly liquid toners developed for use in direct electrostatic printing processes, the D material portion of the organosol is preferably provided with a sufficiently high  $T_g$  such that the organosol exhibits an effective glass transition temperature of from about 15° C. to about 55° C., and the D material portion exhibits a  $T_g$  calculated using the Fox equation, of about 30-55° C.

In one aspect of the present invention, toner particles are provided that are particularly suitable for electrophotographic processes wherein the transfer of the image from the surface of a photoconductor to an intermediate transfer material or directly to a print medium is carried out without film formation on the photoconductor. In this aspect, the D material preferably has a  $T_g$  of at least about 55° C., and more preferably at least about 65° C.

A wide variety of one or more different monomeric, oligomeric and/or polymeric materials can be independently incorporated into the S and D material portions, as desired. Representative examples of suitable materials include free radically polymerized material (also referred to as vinyl copolymers or (meth) acrylic copolymers in some embodiments), polyurethanes, polyester, epoxy, polyamide, polyimide, polysiloxane, fluoropolymer, polysulfone, combinations of these, and the like. Preferred S and D material portions are derived from free radically polymerizable material. In the practice of the present invention, "free radically polymerizable" refers to monomers, oligomers, and/or polymers having functionality directly or indirectly pendant from a monomer, oligomer, or polymer backbone (as the case can be) that participate in polymerization reactions via a free radical mechanism. Representative examples of such functionality includes (meth)acrylate groups, olefinic carbon-carbon double bonds, allyloxy groups, alpha-methyl styrene groups, (meth)acrylamide groups, cyanate ester groups, vinyl ether groups, combinations of these, and the like. The term "(meth)acryl", as used herein, encompasses acryl and/or methacryl.

Free radically polymerizable monomers, oligomers, and/or polymers are advantageously used to form the copolymer

## 12

in that so many different types are commercially available and can be selected with a wide variety of desired characteristics that help provide one or more desired performance characteristics. Free radically polymerizable monomers, oligomers, and/or monomers suitable in the practice of the present invention can include one or more free radically polymerizable moieties.

Representative examples of monofunctional, free radically polymerizable monomers include styrene, alpha-methylstyrene, substituted styrene, vinyl esters, vinyl ethers, N-vinyl-2-pyrrolidone, (meth)acrylamide, vinyl naphthalene, alkylated vinyl naphthalenes, alkoxy vinyl naphthalenes, N-substituted (meth)acrylamide, octyl(meth)acrylate, nonylphenol ethoxylate(meth)acrylate, N-vinyl pyrrolidone, isononyl(meth)acrylate, isobornyl(meth)acrylate, 2-(2-ethoxyethoxy)ethyl(meth)acrylate, 2-ethylhexyl(meth)acrylate, beta-carboxyethyl(meth)acrylate, isobutyl(meth)acrylate, cycloaliphatic epoxide, alpha-epoxide, 2-hydroxyethyl(meth)acrylate, (meth)acrylonitrile, maleic anhydride, itaconic acid, isodecyl(meth)acrylate, lauryl(dodecyl)(meth)acrylate, stearyl(octadecyl)(meth)acrylate, behenyl(meth)acrylate, n-butyl(meth)acrylate, methyl(meth)acrylate, ethyl(meth)acrylate, hexyl(meth)acrylate, (meth)acrylic acid, N-vinylcaprolactam, stearyl(meth)acrylate, hydroxy functional caprolactone ester(meth)acrylate, isoctyl(meth)acrylate, hydroxyethyl(meth)acrylate, hydroxymethyl(meth)acrylate, hydroxypropyl(meth)acrylate, hydroxyisopropyl(meth)acrylate, hydroxyisobutyl(meth)acrylate, tetrahydrofurfuryl(meth)acrylate, isobornyl(meth)acrylate, glycidyl(meth)acrylate, vinyl acetate, combinations of these, and the like.

The monomeric components that are reacted to form the S material portions are, in one embodiment of the present invention, selected to provide the desired  $T_g$  of the S material portion by selection of monomers having  $T_g$ 's within a given range, matched with solubility parameter characteristics. Advantageously, the fusion characteristics and durability property characteristics of the toner and the resulting image formed therefrom can be manipulated by selection of relative  $T_g$ 's of components of S material portions of the amphiphatic copolymer. In this manner, performance characteristics of toner compositions can be readily tailored and/or optimized for use in desired imaging systems. For example, in one embodiment, the average  $T_g$  of the insoluble component is lower than the average  $T_g$  of the soluble components of the S material portion. In a preferred aspect of this embodiment, the average  $T_g$  of the insoluble component is less than about 70° C., and the average  $T_g$  of the soluble components of the S material portion is greater than about 90° C. In another preferred embodiment, the insoluble component has an average  $T_g$  of less than about 0° C., and is from about 1 to about 15% by weight of the S material portion; the soluble component has an average  $T_g$  of greater than about 90° C. and is from about 85 to about 99% by weight of the S material portion.

In another preferred embodiment, the average  $T_g$  of the insoluble component is higher than the average  $T_g$  of the soluble components of the S material portion. In a preferred aspect of this embodiment, the average  $T_g$  of the insoluble component is greater than about 50° C., and the average  $T_g$  of the soluble components of the S material portion is less than about 0° C. In another preferred embodiment, the insoluble component has an average  $T_g$  of greater than about 50° C., and is from about 1 to about 50% by weight of the S material portion; the soluble component has an average  $T_g$  of less than about 0° C., and is from about 50 to about 99% by weight of the S material portion.

## 13

The S material portion is preferably made from (meth)acrylate based monomers and comprises the reaction products of soluble monomers selected from the group consisting of trimethyl cyclohexyl methacrylate; t-butyl methacrylate; n-butyl methacrylate; isobornyl(meth)acrylate; 1,6-Hexanediol di(meth)acrylate; 2-hydroxyethyl methacrylate; lauryl methacrylate; and combinations thereof; and further comprises insoluble components that are the reaction products of monomers selected from the group consisting of ethyl acrylate and ethyl methacrylate.

Preferred copolymers of the present invention can be formulated with one or more radiation curable monomers or combinations thereof that help the free radically polymerizable compositions and/or resultant cured compositions to satisfy one or more desirable performance criteria. For example, in order to promote hardness and abrasion resistance, a formulator can incorporate one or more free radically polymerizable monomer(s) (hereinafter "high  $T_g$  component") whose presence causes the polymerized material, or a portion thereof, to have a higher glass transition temperature,  $T_g$ , as compared to an otherwise identical material lacking such high  $T_g$  component. Preferred monomeric constituents of the high  $T_g$  component generally include monomers whose homopolymers have a  $T_g$  of at least about 50° C., preferably at least about 60° C., and more preferably at least about 75° C. in the cured state. The advantages of incorporating such monomers into the copolymer are further described in assignee's co-pending U.S. patent application filed in the name of Qian et al., U.S. Ser. No. 10/612,765, filed on Jun. 30, 2003, entitled ORGANOSOL INCLUDING HIGH  $T_g$  AMPHIPATHIC COPOLYMERIC BINDER AND LIQUID TONER FOR ELECTROPHOTOGRAPHIC APPLICATIONS; and Qian et al., U.S. Ser. No. 10/612,533, filed on Jun. 30, 2003, entitled ORGANOSOL INCLUDING AMPHIPATHIC COPOLYMERIC BINDER MADE WITH SOLUBLE HIGH  $T_g$  MONOMER AND LIQUID TONERS FOR ELECTROPHOTOGRAPHIC APPLICATIONS for liquid toner compositions, which are hereby incorporated by reference.

An exemplary class of radiation curable monomers that tend to have relatively high  $T_g$  characteristics suitable for incorporation into the high  $T_g$  component generally comprise at least one radiation curable (meth)acrylate monomer and at least one nonaromatic, alicyclic and/or nonaromatic heterocyclic monomer. Isobornyl (meth)acrylate is a specific example of one such monomer. A cured, homopolymer film formed from isobornyl acrylate, for instance, has a  $T_g$  of 110° C. The monomer itself has a molecular weight of 222 g/mole, exists as a clear liquid at room temperature, has a viscosity of 9 centipoise at 25° C., and has a surface tension of 31.7 dynes/cm at 25° C. Additionally, 1,6-Hexanediol di(meth)acrylate is another example of a monomer with high  $T_g$  characteristics. Other examples of preferred high  $T_g$  components include trimethyl cyclohexyl methacrylate; t-butyl methacrylate; n-butyl methacrylate. Combinations of high  $T_g$  components for use in both the S material portion and the soluble polymer are specifically contemplated, together with anchor grafting groups such as provided by use of HEMA subsequently reacted with TMI.

Copolymers of the present invention can be prepared by free-radical polymerization methods known in the art, including but not limited to bulk, solution, and dispersion polymerization methods. The resultant copolymers can have a variety of structures including linear, branched, three dimensionally networked, graft-structured, combinations thereof, and the like. A preferred embodiment is a graft copolymer comprising one or more oligomeric and/or poly-

## 14

meric arms attached to an oligomeric or polymeric backbone. In graft copolymer embodiments, the S material portion or D material portion materials, as the case can be, can be incorporated into the arms and/or the backbone.

Any number of reactions known to those skilled in the art can be used to prepare a free radically polymerized copolymer having a graft structure. Common grafting methods include random grafting of polyfunctional free radicals; copolymerization of monomers with macromonomers; ring-opening polymerizations of cyclic ethers, esters, amides or acetals; epoxidations; reactions of hydroxyl or amino chain transfer agents with terminally-unsaturated end groups; esterification reactions (i.e., glycidyl methacrylate undergoes tertiary-amine catalyzed esterification with methacrylic acid); and condensation polymerization.

Representative methods of forming graft copolymers are described in U.S. Pat. Nos. 6,255,363; 6,136,490; and 5,384,226; and Japanese Published Patent Document No. 05-119529, incorporated herein by reference. Representative examples of grafting methods are also described in sections 3.7 and 3.8 of Dispersion Polymerization in Organic Media, K. E. J. Barrett, ed., (John Wiley; New York, 1975) pp. 79-106, also incorporated herein by reference.

In preferred embodiments, the copolymer is polymerized in situ in the desired liquid carrier, as this yields substantially monodisperse copolymeric particles suitable for use in toner compositions. The resulting organosol is then preferably mixed with at least one visual enhancement additive and optionally one or more other desired ingredients to form a liquid toner. During such combination, ingredients comprising the visual enhancement particles and the copolymer will tend to self-assemble into composite particles having solvated (S) portions and dispersed (D) portions. Specifically, it is believed that the D material of the copolymer will tend to physically and/or chemically interact with the surface of the visual enhancement additive, while the S material helps promote dispersion in the carrier.

Representative examples of grafting methods also can use an anchoring group. The function of the anchoring group is to provide a covalently bonded link between the core part of the copolymer (the D material) and the soluble shell component (the S material). Preferred amphiphilic copolymers are prepared by first preparing an intermediate S material portion comprising reactive functionality by a polymerization process, and subsequently reacting the available reactive functionalities with a graft anchoring compound. The graft anchoring compound comprises a first functionality that can be reacted with the reactive functionality on the intermediate S material portion, and a second functionality that is a polymerizable reactive functionality that can take part in a polymerization reaction. After reaction of the intermediate S material portion with the graft anchoring compound, a polymerization reaction with selected monomers can be carried out in the presence of the S material portion to form a D material portion having one or more S material portions grafted thereto.

Suitable monomers containing anchoring groups include: adducts of alkenylazlactone comonomers with an unsaturated nucleophile containing hydroxy, amino, or mercaptan groups, such as 2-hydroxyethylmethacrylate, 3-hydroxypropylmethacrylate, 2-hydroxyethylacrylate, pentaerythritol triacrylate, 4-hydroxybutylvinylether, 9-octadecen-1-ol, cinnamyl alcohol, allyl mercaptan, methylallylamine; and azlactones, such as 2-alkenyl-4,4-dialkylazlactone.

The preferred methodology described above accomplishes grafting via attaching an ethylenically-unsaturated isocyanate (e.g., dimethyl-m-isopropenyl benzylisocyanate,

## 15

TMI, available from CYTEC Industries, West Paterson, N.J.; or isocyanatoethyl methacrylate, IEM) to hydroxyl groups in order to provide free radically reactive anchoring groups.

A preferred method of forming a graft copolymer of the present invention involves three reaction steps that are carried out in a suitable substantially nonaqueous liquid carrier in which resultant S material is soluble while D material is dispersed or insoluble.

In a first preferred step, a hydroxyl functional, free radically polymerized oligomer or polymer is formed from one or more monomers, wherein at least one of the monomers has pendant hydroxyl functionality. Preferably, the hydroxyl functional monomer constitutes about 1 to about 30, preferably about 2 to about 10 percent, most preferably 3 to about 5 percent by weight of the monomers used to form the oligomer or polymer of this first step. This first step is preferably carried out via solution polymerization in a substantially nonaqueous solvent in which the monomers and the resultant polymer are soluble. For instance, using the Hildebrand solubility data in Table 1, monomers such as octadecyl methacrylate, octadecyl acrylate, lauryl acrylate, and lauryl methacrylate are suitable for this first reaction step when using an oleophilic solvent such as heptane or the like.

In a second reaction step, all or a portion of the hydroxyl groups of the soluble polymer are catalytically reacted with an ethylenically unsaturated aliphatic isocyanate (e.g. meta-isopropenylidimethylbenzyl isocyanate commonly known as TMI or isocyanatoethyl methacrylate, commonly known as IEM) to form pendant free radically polymerizable functionality which is attached to the oligomer or polymer via a polyurethane linkage. This reaction can be carried out in the same solvent, and hence the same reaction vessel, as the first step. The resultant double-bond functionalized polymer generally remains soluble in the reaction solvent and constitutes the S material portion material of the resultant copolymer, which ultimately will constitute at least a portion of the solvatable portion of the resultant triboelectrically charged particles.

The resultant free radically reactive functionality provides grafting sites for attaching D material and optionally additional S material to the polymer. In a third step, these grafting site(s) are used to covalently graft such material to the polymer via reaction with one or more free radically reactive monomers, oligomers, and or polymers that are initially soluble in the solvent, but then become insoluble as the molecular weight of the graft copolymer. For instance, using the Hildebrand solubility parameters in Table 1, monomers such as e.g. methyl (meth)acrylate, ethyl (meth)acrylate, t-butyl methacrylate and styrene are suitable for this third reaction step when using an oleophilic solvent such as heptane or the like.

The product of the third reaction step is generally an organosol comprising the resultant copolymer dispersed in the reaction solvent, which constitutes a substantially nonaqueous liquid carrier for the organosol. At this stage, it is believed that the copolymer tends to exist in the liquid carrier as discrete, monodisperse particles having dispersed (e.g., substantially insoluble, phase separated) portion(s) and solvated (e.g., substantially soluble) portion(s). As such, the solvated portion(s) help to sterically-stabilize the dispersion of the particles in the liquid carrier. It can be appreciated that the copolymer is thus advantageously formed in the liquid carrier *in situ*.

Before further processing, the copolymer particles can remain in the reaction solvent. Alternatively, the particles

## 16

can be transferred in any suitable way into fresh solvent that is the same or different so long as the copolymer has solvated and dispersed phases in the fresh solvent. In either case, the resulting organosol is then converted into toner particles by mixing the organosol with at least one visual enhancement additive. Optionally, one or more other desired ingredients also can be mixed into the organosol before and/or after combination with the visual enhancement particles. During such combination, it is believed that ingredients comprising the visual enhancement additive and the copolymer will tend to self-assemble into composite particles having a structure wherein the dispersed phase portions generally tend to associate with the visual enhancement additive particles (for example, by physically and/or chemically interacting with the surface of the particles), while the solvated phase portions help promote dispersion in the carrier.

The visual enhancement additive(s) generally may include any one or more fluid and/or particulate materials that provide a desired visual effect when toner particles incorporating such materials are printed onto a receptor. Examples include one or more colorants, fluorescent materials, pearlescent materials, iridescent materials, metallic materials, flip-flop pigments, silica, polymeric beads, reflective and non-reflective glass beads, mica, combinations of these, and the like. The amount of visual enhancement additive coated on binder particles may vary over a wide range. In representative embodiments, a suitable weight ratio of copolymer to visual enhancement additive is from 1/1 to 20/1, preferably from 2/1 to 10/1 and most preferably from 4/1 to 8/1.

Useful colorants are well known in the art and include materials listed in the Colour Index, as published by the Society of Dyers and Colourists (Bradford, England), including dyes, stains, and pigments. Preferred colorants are pigments which may be combined with ingredients comprising the binder polymer to form dry toner particles with structure as described herein, are at least nominally insoluble in and nonreactive with the carrier liquid, and are useful and effective in making visible the latent electrostatic image. It is understood that the visual enhancement additive(s) may also interact with each other physically and/or chemically, forming aggregations and/or agglomerates of visual enhancement additives that also interact with the binder polymer. Examples of suitable colorants include: phthalocyanine blue (C.I. Pigment Blue 15:1, 15:2, 15:3 and 15:4), monoarylide yellow (C.I. Pigment Yellow 1, 3, 65, 73 and 74), diarylide yellow (C.I. Pigment Yellow 12, 13, 14, 17 and 83), arylamide (Hansa) yellow (C.I. Pigment Yellow 10, 97, 105 and 111), isoindoline yellow (C.I. Pigment Yellow 138), azo red (C.I. Pigment Red 3, 17, 22, 23, 38, 48:1, 48:2, 52:1, and 52:179), quinacridone magenta (C.I. Pigment Red 122, 202 and 209), laked rhodamine magenta (C.I. Pigment Red 81:1, 81:2, 81:3, and 81:4), and black pigments such as finely divided carbon (Cabot Monarch 120, Cabot Regal 300R, Cabot Regal 350R, Vulcan X72, and Aztech EK 8200), and the like.

The toner particles of the present invention may additionally comprise one or more additives as desired. Additional additives include, for example, UV stabilizers, mold inhibitors, bactericides, fungicides, antistatic agents, anticaking agents, gloss modifying agents, other polymer or oligomer material, antioxidants, and the like.

Charge directors can be used in any liquid toner process, and particularly can be used for electrostatic transfer of toner particles or transfer assist materials. The charge director typically provides the desired uniform charge polarity of the

toner particles. In other words, the charge director acts to impart an electrical charge of selected polarity onto the toner particles as dispersed in the carrier liquid. Preferably, the charge director is coated on the outside of the binder particle. Alternatively or additionally, the charge director can be incorporated into the toner particles using a wide variety of methods, such as copolymerizing a suitable monomer with the other monomers to form a copolymer, chemically reacting the charge director with the toner particle, chemically or physically adsorbing the charge director onto the toner particle, or chelating the charge director to a functional group incorporated into the toner particle.

The preferred amount of charge director or charge control additive for a given toner formulation will depend upon a number of factors, including the composition of the polymer binder. Preferred polymeric binders are graft amphiphilic copolymers. The preferred amount of charge director or charge control additive when using an organosol binder particle further depends on the composition of the S material portion of the graft copolymer, the composition of the organosol, the molecular weight of the organosol, the particle size of the organosol, the core/shell ratio of the graft copolymer, the pigment used in making the toner, and the ratio of organosol to pigment. In addition, preferred amounts of charge director or charge control additive will also depend upon the nature of the electrophotographic imaging process, particularly the design of the developing hardware and photoreceptive element. It is understood, however, that the level of charge director or charge control additive can be adjusted based on a variety of parameters to achieve the desired results for a particular application.

Any number of charge directors such as those described in the art can be used in the liquid toners or transfer assist materials of the present invention in order to impart a negative electrical charge onto the toner particles. For example, the charge director can be lecithin, oil-soluble petroleum sulfonates (such as neutral Calcium Petronate<sup>TM</sup>, neutral Barium Petronate<sup>TM</sup>, and basic Barium Petronate<sup>TM</sup>, manufactured by Sonneborn Division of Witco Chemical Corp., New York, N.Y.), polybutylene succinimides (such as OLOA<sup>TM</sup> 1200 sold by Chevron Corp., and Amoco 575), and glyceride salts (such as sodium salts of phosphated mono- and diglycerides with unsaturated and saturated acid substituents as disclosed in U.S. Pat. No. 4,886,726 to Chan et al.). A preferred type of glyceride charge director is the alkali metal salt (e.g., Na) of a phosphoglyceride. A preferred example of such a charge director is Emphos<sup>TM</sup> D70-30C, Witco Chemical Corp., New York, N.Y., which is a sodium salt of phosphated mono- and diglycerides.

Any number of charge directors such as those described in the art can be used in the liquid toners or transfer assist materials of the present invention in order to impart a positive electrical charge onto the toner particles. For example, the charge director can be introduced in the form of metal salts consisting of polyvalent metal ions and organic anions as the counterion. Suitable metal ions include Ba(II), Ca(II), Mn(II), Zn(II), Zr(IV), Cu(II), Al(III), Cr(III), Fe(II), Fe(III), Sb(III), Bi(III) Co(II), La(III), Pb(II), Mg(II), Mo(III), Ni(II), Ag(I), Sr(II), Sn(IV), V(V), Y(III) and Ti(IV). Suitable organic anions include carboxylates or sulfonates derived from aliphatic or aromatic carboxylic or sulfonic acids, preferably aliphatic fatty acids such as stearic acid, behenic acid, neodecanoic acid, diisopropylsalicylic acid, octanoic acid, abietic acid, naphthenic acid, octanoic acid, lauric acid, tallic acid, and the like. Preferred positive charge directors are the metallic carboxylates (soaps), such

as those described in U.S. Pat. No. 3,411,936. A particularly preferred positive charge director is zirconium 2-ethyl hexanoate.

The conductivity of a liquid toner composition can be used to describe the effectiveness of the toner in developing electrophotographic images. A range of values from  $1 \times 10^{-11}$  Mhos/cm to  $3 \times 10^{-10}$  Mhos/cm is considered advantageous to those of skill in the art. High conductivities generally indicate inefficient association of the charges on the toner particles and is seen in the low relationship between current density and toner deposited during development. Low conductivities indicate little or no charging of the toner particles and lead to very low development rates. The use of charge directors matched to adsorption sites on the toner particles is a common practice to ensure sufficient charge associates with each toner particle.

Other additives can also be added to the formulation in accordance with conventional practices. These include one or more of UV stabilizers, mold inhibitors, bactericides, fungicides, antistatic agents, gloss modifying agents, other polymer or oligomer material, antioxidants, and the like.

The particle size of the resultant charged toner particles can impact the imaging, fusing, resolution, and transfer characteristics of the toner composition incorporating such particles. Preferably, the volume mean particle diameter (determined with laser diffraction) of the toner particles is in the range of about 0.05 to about 50.0 microns, more preferably in the range of about 1.5 to about 10 microns, most preferably in the range of about 3 to about 5 microns. In electrophotographic and electrographic processes, an electrostatic image is formed on the surface of a photoreceptive element or dielectric element, respectively. The photoreceptive element or dielectric element can be an intermediate transfer drum or belt or the substrate for the final toned image itself, as described by Schmidt, S. P. and Larson, J. R. in *Handbook of Imaging Materials* Diamond, A. S., Ed: Marcel Dekker: New York; Chapter 6, pp 227-252, and U.S. Pat. Nos. 4,728,983, 4,321,404, and 4,268,598.

In electrography, a latent image is typically formed by (1) placing a charge image onto the dielectric element (typically the receiving substrate) in selected areas of the element with an electrostatic writing stylus or its equivalent to form a charge image, (2) applying toner to the charge image, and (3) fixing the toned image. An example of this type of process is described in U.S. Pat. No. 5,262,259. Images formed by the present invention can be of a single color or a plurality of colors. Multicolor images can be prepared by repetition of the charging and toner application steps.

In electrophotography, the electrostatic image is typically formed on a drum or belt coated with a photoreceptive element by (1) uniformly charging the photoreceptive element with an applied voltage, (2) exposing and discharging portions of the photoreceptive element with a radiation source to form a latent image, (3) applying a toner to the latent image to form a toned image, and (4) transferring the toned image through one or more steps to a final receptor sheet. In some applications, it is sometimes desirable to fix the toned image using a heated pressure roller or other fixing methods known in the art.

While the electrostatic charge of either the toner particles or photoreceptive element can be either positive or negative, electrophotography as employed in the present invention is preferably carried out by dissipating charge on a positively charged photoreceptive element. A positively-charged toner is then applied to the regions in which the positive charge was dissipated using a liquid toner development technique.

The substrate for receiving the image from the photoreceptive element can be any commonly used receptor material, such as paper, coated paper, polymeric films and primed or coated polymeric films. Polymeric films include polyesters and coated polyesters, polyolefins such as polyethylene or polypropylene, plasticized and compounded polyvinyl chloride (PVC), acrylics, polyurethanes, polyethylene/acrylic acid copolymer, and polyvinyl butyral. The polymer film can be coated or primed, e.g. to promote toner adhesion.

In electrophotographic processes, the toner composition preferably is provided at a solids content of about 1-30%. In electrostatic processes, the toner composition preferably is provided at a solids content of 3-15%.

These and other aspects of the present invention are demonstrated in the illustrative examples that follow.

## EXAMPLES

### A. Test Methods and Apparatus

#### Percent Solids

In the following examples, percent solids of the graft stabilizer solutions and the organosol and liquid toner dispersions were determined thermo-gravimetrically by drying in an aluminum weighing pan an originally-weighed sample at 160° C. for two hours for graft stabilizer, three hours for organosol, and two hours for liquid toner dispersions, weighing the dried sample, and calculating the percentage ratio of the dried sample weight to the original sample weight, after accounting for the weight of the aluminum weighing pan. Approximately two grams of sample were used in each determination of percent solids using this thermo-gravimetric method.

#### Molecular Weight

In the practice of the invention, molecular weight is normally expressed in terms of the weight average molecular weight, while molecular weight polydispersity is given by the ratio of the weight average molecular weight to the number average molecular weight. Molecular weight parameters were determined with gel permeation chromatography (GPC) using a Hewlett Packard Series II 1190 Liquid Chromatograph made by Agilent Industries (formerly Hewlett Packard, Palo Alto, Calif.) (using software HPLC Chemstation Rev A.02.02 1991-1993 395). Tetrahydrofuran was used as the carrier solvent. The three columns used in the Liquid Chromatograph were Jordi Gel Columns (DVB 1000A, and DVB10000A and DVB100000A; Jordi Associates, Inc., Bellingham, Mass.). Absolute weight average molecular weight were determined using a Dawn DSP-F light scattering detector (software by Astra v.4.73.04 1994-1999) (Wyatt Technology Corp., Santa Barbara, Calif.), while polydispersity was evaluated by ratioing the measured weight average molecular weight to a value of number average molecular weight determined with an Optilab DSP Interferometric refractometer detector (Wyatt Technology Corp., Santa Barbara, Calif.).

#### Glass Transition Temperature

For the glass transition temperatures measurement, a graft stabilizer sample was prepared by washing the polymer mixture with acetone and/or methanol followed by drying at 100° C. for 2 hours while an organosol sample was prepared by drying the polymer mixture in an oven at 160° C. for 3 hours. The glass transition temperatures of the dried polymer samples were then measured using a Differential Scanning Calorimeter (TA Instruments Model 2929, New Castle, Del.) equipped with a DSC refrigerated cooling system (-60° C.

minimum temperature limit), and dry helium and nitrogen exchange gases. The calorimeter ran on a Thermal Analyst 2100 workstation with version 8.10B software. An empty aluminium pan was used as the reference. Each sample was evaluated using 10° C./min heating and cooling rates with a 5-10 min isothermal bath at the end of each heating or cooling ramp. Each sample was heated three to five times and the values for  $T_g$  were reported from either the third or fourth heat ramp. Samples for which a  $T_g$  measurement could not be obtained had their  $T_g$ s calculated using the Fox equation as described above.

#### Particle Size

The organosol (and liquid ink) particle size distributions were determined using a Horiba LA-920 laser diffraction particle size analyzer (commercially obtained from Horiba Instruments, Inc, Irvine, Calif.) using Norpar™ 12 fluid that contains 0.1% Aerosol OT (dioctyl sodium sulfosuccinate, sodium salt, Fisher Scientific, Fairlawn, N.J.) surfactant.

Prior to the measurements, samples were pre-diluted to approximately 1% (w/w) by the solvent (i.e., Norpar™12), and were sonicated for 6 minutes in a Probe VirSonic sonicator (Model-550 by The VirTis Company, Inc., Gardiner, N.Y.). The pre-diluted samples were further diluted by approximately 1/500 by volume during the measurements and were sonicated for one minute before data was collected. Sonication on the Horiba LA-920 was operated at 150 watts and 20 kHz. The particle size was expressed on a number-average basis in order to provide an indication of dominance of the fundamental (primary) particle size of the particles or was expressed on a volume-average basis in order to provide an indication of dominance of the coalesced primary particle aggregate size of the particles.

#### Conductivity

The liquid toner conductivity (bulk conductivity,  $k_b$ ) was determined at approximately 18 Hz using a Scientifica Model 627 conductivity meter (Scientifica Instruments, Inc., Princeton, N.J.). In addition, the free (liquid dispersant) phase conductivity ( $k_f$ ) in the absence of toner particles was also determined. Toner particles were removed from the liquid medium by centrifugation at 10° C. for 1 hour at 7,500 rpm (6,110 relative centrifugal force) in a Jouan MR1822 centrifuge (Winchester, Va.). The supernatant liquid was then carefully decanted, and the conductivity of this liquid was measured using a Scientifica Model 627 conductance meter. The percentage of free phase conductivity relative to the bulk toner conductivity was then determined (i.e.  $(k_f/k_b) \%$ ).

#### Mobility

Toner particle electrophoretic mobility (dynamic mobility) was measured using a Matec MBS-8000 Electrokinetic Sonic Amplitude Analyzer (Matec Applied Sciences, Inc., Hopkinton, Mass.). Unlike electrokinetic measurements based upon microelectrophoresis, the MBS-8000 instrument has the advantage of requiring no dilution of the toner sample in order to obtain the mobility value. Thus, it was possible to measure toner particle dynamic mobility at solids concentrations actually preferred in printing. The MBS-8000 measures the response of charged particles to high frequency (1.2 MHz) alternating (AC) electric fields. In a high frequency AC electric field, the relative motion between charged toner particles and the surrounding dispersion medium (including counter-ions) generates an ultrasonic wave at the same frequency of the applied electric field. The amplitude of this ultrasonic wave at 1.2 MHz can be measured using a piezoelectric quartz transducer; this

21

electrokinetic sonic amplitude (ESA) is directly proportional to the low field AC electrophoretic mobility of the particles. The particle zeta potential can then be computed by the instrument from the measured dynamic mobility and the known toner particle size, liquid dispersant viscosity, and liquid dielectric constant.

Q/M

The charge per mass measurement (Q/m) was measured using an apparatus that consists of a conductive metal plate, a glass plate coated with Indium Tin Oxide (ITO), a high voltage power supply, an electrometer, and a personal computer (PC) for data acquisition. A 1% solution of ink was placed between the conductive plate and the ITO coated glass plate. An electrical potential of known polarity and magnitude was applied between the ITO coated glass plate and the metal plate, generating a current flow between the plates and through wires connected to the high voltage power supply. The electrical current was measured 100 times a second for 20 seconds and recorded using the PC. The applied potential causes the charged toner particles to migrate towards the plate (electrode) having opposite polarity to that of the charged toner particles. By controlling the polarity of the voltage applied to the ITO coated glass plate, the toner particles may be made to migrate to that plate.

The ITO coated glass plate was removed from the apparatus and placed in an oven for at least 2 hours at 55° C. to dry the plated ink completely. After drying, the ITO coated glass plate containing the dried ink film was weighed. The ink was then removed from the ITO coated glass plate using a cloth wipe impregnated with Norpar™12, and the clean ITO glass plate was weighed again. The difference in mass between the dry ink coated glass plate and the clean glass plate is taken as the mass of ink particles (m) deposited during the 20 second plating time. The electrical current values were used to obtain the total charge carried by the toner particles (Q) over the 20 seconds of plating time by integrating the area under a plot of current vs. time using a curve-fitting program (e.g. TableCurve 2D from Systat Software Inc.). The charge per mass (Q/m) was then determined by dividing the total charge carried by the toner particles by the dry plated ink mass.

#### Print Testing

In the following examples, toner was printed onto final image receptors using the following methodology:

A light-sensitive temporary image receptor (organic photoreceptor or "OPC") was charged with a uniform positive charge of approximately 850 volts. The positively charged surface of the OPC was image-wise irradiated with a scanning infrared laser module in order to reduce the charge wherever the laser struck the surface. Typical charge-reduced values were between 50 volts and 100 volts.

A developer apparatus was then utilized to apply the toner particles to the OPC surface. The developer apparatus included the following elements: liquid toner, a conductive rubber developer roller in contact with the OPC, an insulative foam cleaning roller in contact with the developer roller surface, a conductive deposition roller, a conductive metering roll in contact with the developer roller, and an insulative foam ink pumping roller. The contact area between the developer roller and the OPC is referred to as the "developing nip." The conductive deposition roller was positioned with its roller axis parallel to the developer roller axis and its surface arranged to be approximately 150 microns from the surface of the developer roller, thereby forming a deposition gap.

22

During development, the ink pumping roller supplied liquid ink to the gap between the deposition roller and the developer roller. A toner film was initially plated to the developer roller surface by applying a voltage of approximately 600 volts to the developer roller and applying a voltage of approximately 800 volts to both the deposition and metering rollers. The 200 volt difference between the developer and deposition roller caused the positively charged toner particles to migrate in the deposition nip to the surface of the developer roller. The metering roller, which is biased to approximately 800 volts, removed excess liquid from the developer roller surface.

The surface of the developer roller now contained a uniformly thick layer of toner at approximately 25% (w/w) solids. As this toner layer passed through the developing nip, toner was transferred from the developer roller to the latent image areas. The approximate 500 volt difference between the developer roller and the latent image area caused the positively charged toner particles to develop to the OPC surface. At the exit of the developing nip, the OPC contained a toner image and the developer roller contained a negative of that toner image which was then cleaned from the developer roller surface by the rotating foam cleaning roller.

The developed image on the OPC was subsequently electrostatically transferred to an Intermediate Transfer Belt (ITB) with an electrical bias in the range of -800 to -2000 volts applied to a conductive rubber roller pressing the ITB to the OPC surface. Transfer to the final image receptor was accomplished with electrostatically-assisted offset transfer by forcibly applying a conductive, biased rubber transfer roller behind the image receptor, pressing the imaged ITB between the final image receptor and a grounded, conductive metal transfer backup roller. The transfer roller is typically biased in the range of -1200 to -3000 volts.

Prints were generated, using the method as described above, having a first solid block of magenta toner printed to the page, then a second solid block of cyan toner printed to the same page. The two solid blocks of color were applied such that at least a portion of the cyan block overlapped at least a portion of the magenta block, creating a two-color overlay area that was "blue." The entire imaged page, having a magenta area, a cyan area and a blue area were fused as described below.

#### Fusing Test

The image was fixed to the final image receptor (paper) using a two station fusing unit attached to the printing device described above. The fusing unit was mounted directly above the paper exit. The fusing unit was comprised of two sets of rollers (two stations), with each set of rollers having a different coating. The imaged page was passed between each set of rollers such that for each set of rollers, one roller contacted the image surface and one contacted the backside (non-imaged side) of the page.

Both set of rollers contained silicone rubber for the base. For each set of rollers, the roller that contacted the image surface had a Shore A 10 durometer rubber base; the backup roller had a Shore A 20 durometer rubber base. The first set of rollers between which the imaged receptor passed may be set to a lower temperature than the second set and had a dimethyl siloxane coating on both rollers to alleviate offset when contacting the liquid toner. The second set of rollers between which the imaged receptor passed are capable of being set to a high temperature and were covered with a molded in place Teflon® sleeve to fuse the semi-dried liquid toner. Each roller contained a 600W/138 volt halogen lamp for a heat source. An IR probe was used to read the

temperature of the top and bottom image contacting roller. Additional information is given in the chart below

| Summary of Fusing Conditions |                                     |                     |                     |                       |
|------------------------------|-------------------------------------|---------------------|---------------------|-----------------------|
| Roller set                   | Amount of force between the rollers | Maximum Temperature | Minimum Temperature | Fusing (Roller) Speed |
| 1 <sup>st</sup> pair         | 20 PSI                              | 200° C.             | 100° C.             | 4.9 in/sec            |
| 2 <sup>nd</sup> pair         | 23 PSI                              | 200° C.             | 100° C.             | 4.9 in/sec            |

Both rollers sets were the set at the same temperature in 10° C. increments from 100° C. to 200° C. for each ink evaluated. If the fusing lamps overheated the rollers, they were allowed to cool down until the testing temperature was reached. If the rollers were too cool, they were allowed to warm up and cool back down to the evaluation temperature. If conditions were run which exhibited offset, the rollers were cleaned with Norpar 12 before the next temperature setting was run.

All fused images were subjected to image durability testing, which is described below.

#### Fused Image Erasure Resistance:

In these experiments, the cyan and magenta overlay area (the "blue" region) was tested for fused image durability. The evaluation took place as soon as possible after fusing. This test is used to determine image durability when a printed image is subjected to abrasion from materials such as other paper, linen cloth, and pencil erasers.

In order to quantify the resistance of the printed ink to erasure forces after fusing, an erasure test has been defined. This erasure test consists of using a device called a Crockmeter to abrade the inked and fused areas with a linen cloth loaded against the ink with a known and controlled force. A standard test procedure followed generally by the inventors is defined in ASTM #F 1319-94 (American Standard Test Methods). The Crockmeter used in this testing was an AATCC Crockmeter Model CM1 manufactured by Atlas Electric Devices Company, Chicago, Ill. 60613.

A piece of linen cloth (WW-3009 Super Clean Wiper, available from WOOGIN Act. Corp., Republic of Korea) is affixed to the Crockmeter probe; the probe is placed onto the printed surface with a controlled force and caused to slew back and forth on the printed surface a prescribed number of times (in this case, 10 times by the turning of a small crank with 5 full turns at two slews per turn). The prepared samples are of sufficient length so that during the slewing, the linen-covered Crockmeter probe head never leaves the printed surface by crossing the ink boundary and slewing onto the paper surface.

For this Crockmeter, the head weight was 934 grams, which is the weight placed on the ink during the 10-slew test, and the area of contact of the linen-covered probe head with the ink was 1.76 cm<sup>2</sup>. The results of this test are obtained as described in the standard test method, by determining the optical density of the printed area before the abrasion measured on paper and the optical density after the abrasion measured on linen cloth. The difference between the two numbers is divided by the original density and multiplied by 100% to obtain the fused image erasure resistance.

#### Optical Density and Color Purity

To measure optical density and color purity a GRETAG SPM 50 LT meter was used. The meter is made by Gretag Limited, CH-8105 Regensdorf, Switzerland. The meter has

several different functions through different modes of operations, selected through different buttons and switches. When a function (optical density, for example) is selected, the measuring orifice of the meter is placed on a background, or a non-imaged portion of the imaged substrate in order to "zero" it. It is then placed on the designated color patch and the measurement button is activated. The optical densities of the various color components of the color patch (in this case, Cyan (C), Magenta (M), Yellow (Y), and Black (K)) will then be displayed on the screen of the meter. The value of each specific component is then used as the optical density for that component of the color patch. For instance, where a color patch is only cyan, the optical density reading may be listed as simply the value on the screen for C.

#### 15 Material Abbreviations

The following abbreviations are used in the examples:  
EA: Ethyl acrylate (available from Aldrich Chemical Co., Milwaukee, Wis.)

EMA: Ethyl methacrylate (available from Aldrich Chemical Co., Milwaukee, Wis.)

HEMA: 2-Hydroxyethyl methacrylate (available from Aldrich Chemical Co., Milwaukee, Wis.)

LMA: Lauryl methacrylate (available from Aldrich Chemical Co., Milwaukee, Wis.)

TCHMA: Trimethyl cyclohexyl methacrylate (available from Ciba Specialty Chemical Co., Suffolk, Va.)

TMI: Dimethyl-m-isopropenyl benzyl isocyanate (available from CYTEC Industries, West Paterson, N.J.)

V-601: Dimethyl 2,2'-azobisisobutyrate (an initiator available as V-601 from WAKO Chemicals U.S.A., Richmond, Va.)

V-64: 2,2'-azobisisobutyronitrile (an initiator available as V-64 from WAKO Chemicals U.S.A., Richmond, Va.)

DBTDL: Dibutyl tin dilaurate (a catalyst available from Aldrich Chemical Co., Milwaukee, Wis.)

Zirconium HEX-CEM: (metal soap, zirconium tetraoctoate, available from OMG Chemical Company, Cleveland, Ohio)

#### 40 Nomenclature

In the following examples, the compositional details of each copolymer will be summarized by ratioing the weight percentages of monomers used to create the copolymer. The grafting site composition is expressed as a weight percentage of the monomers comprising the copolymer or copolymer precursor, as the case may be. For example, a graft stabilizer (precursor to the S portion of the copolymer) designated TCHMA/HEMA-TMI (97/3-4.7% w/w) is made by copolymerizing, on a relative basis, 97 parts by weight TCHMA and 3 parts by weight HEMA, and this hydroxy functional polymer was reacted with 4.7 parts by weight of TMI.

Similarly, a graft copolymer organosol designated TCHMA/HEMA-TMI//EMA (97/3-4.7//100% (w/w)) is made by copolymerizing the designated graft stabilizer (TCHMA/HEMA-TMI (97/3-4.7% (w/w))) (S portion or shell) with the designated core monomer EMA (D portion or core, 100% (w/w) EMA) at a specified ratio of D/S (core/shell) determined by the relative weights reported in the examples.

#### 60 Example 1 (Comparative)

A clean 50 gallon reactor was equipped with a condenser, a thermocouple connected to a digital temperature controller, a nitrogen inlet tube connected to a source of dry nitrogen and a mixer. To the reactor was charged with 195

lbs of Norpar<sup>TM</sup>12 by vacuum. The vacuum was then broken and a flow of 1 CFH (cubic foot per hour) of nitrogen applied and the agitation was started at 70 RPM. 66.4 lbs of TCHMA was added and the container rinsed with 2.7 lbs of Norpar<sup>TM</sup>12. 2.10 lbs of 98% (w/w) HEMA was added and the container rinsed with 1.37 lbs of Norpar<sup>TM</sup>12. Finally 0.86 lb of V-601 was added and the container rinsed with 0.2 lb of Norpar<sup>TM</sup>12. A full vacuum was then applied for 10 minutes, and then broken by a nitrogen blanket. A second vacuum was pulled for 10 minutes, and then agitation stopped to verify that no bubbles were coming out of the solution. The vacuum was then broken with a nitrogen blanket and a light flow of nitrogen of 1 CFH was applied. Agitation was resumed at 75 RPM and the mixture was heated to 75° C. and held for 4 hours. The conversion was quantitative.

The mixture was heated to 100° C. and held at that temperature for 1 hour to destroy any residual V-601, and then was cooled down to 70° C. The nitrogen inlet tube was then removed, and 0.11 lb of 95% (w/w) DBTDL was added to the mixture using 1.37 lbs of Norpar<sup>TM</sup>12 to rinse container, followed by 3.23 lbs of TMI. The TMI was added drop wise over the course of approximately 5 minutes while stirring the reaction mixture and the container was rinsed with 1.4 lbs of Norpar<sup>TM</sup>12. The mixture was allowed to react at 70° C. for 2 hours, at which time the conversion was quantitative.

The cooled mixture was a viscous, transparent liquid containing no visible insoluble matter. The percent solids of the liquid mixture was determined to be 26.2% (w/w) using the thermo-gravimetric method described above. Subsequent determination of molecular weight was made using the GPC method described above; the copolymer had a  $M_w$  of 251,300 Da and  $M_w/M_n$  of 2.8 based on two independent measurements. The measured glass transition temperature of the polymer was 123.0° C., as determined by DSC using the method described above. The product was a copolymer of TCHMA and HEMA containing random side chains of TMI and was designated herein as TCHMA/HEMA-TMI (97/3-4.7% w/w). It can be used to make an organosol.

#### Example 2 (Comparative)

Using the method and apparatus of Example 1, 194 lbs of Norpar<sup>TM</sup>12 was charged to the reactor by vacuum. The vacuum was then broken and a flow of 1 CFH of nitrogen applied and the agitation was started at 70 RPM. 66.4 lbs of LMA was added and the container rinsed with 2.5 lbs of Norpar<sup>TM</sup>12. 2.10 lbs of 98% (w/w) HEMA was added and the container rinsed with 1.37 lbs of Norpar<sup>TM</sup>12. Finally 0.52 lb of V-64 was added and the container rinsed with 0.2 lb of Norpar<sup>TM</sup>12. A full vacuum was then applied for 10 minutes, and then broken by a nitrogen blanket. A second vacuum was pulled for 10 minutes, and then agitation stopped to verify that no bubbles were coming out of the solution. The vacuum was then broken with a nitrogen blanket and a light flow of nitrogen of 1 CFH (cubic foot per hour) was applied. Agitation was resumed at 75 RPM and the mixture was heated to 70° C. and held for 16 hours. The conversion was quantitative.

The mixture was heated to 90° C. and held at that temperature for 1 hour to destroy any residual V-64, and then was cooled down to 70° C. The nitrogen inlet tube was then removed, and 1.06 lbs of 95% (w/w) DBTDL was added to the mixture using 1.37 lbs of Norpar<sup>TM</sup>12 to rinse container, followed by 3.23 lbs of TMI. The TMI was added drop wise over the course of approximately 5 minutes while stirring the reaction mixture and the container was rinsed with 1.4

lbs of Norpar<sup>TM</sup>12. The mixture was allowed to react at 70° C. for 6 hours, at which time the conversion was quantitative.

The cooled mixture was a viscous, transparent liquid containing no visible insoluble matter. The percent solids of the liquid mixture was determined to be 26.6% (w/w) using the thermo-gravimetric method described above. Subsequent determination of molecular weight was made using the GPC method described above; the copolymer had a  $M_w$  of 261,950 Da and  $M_w/M_n$  of 2.4 based upon two independent measurements. The calculated glass transition temperature of the polymer was -63° C., as determined by the Fox equation described above. The product was a copolymer of LMA and HEMA containing random side chains of TMI and was designated herein as LMA/HEMA-TMI (97/3-4.7% w/w). It can be used to make an organosol.

#### Example 3

20 A 5000 ml 3-neck round flask equipped with a condenser, a thermocouple connected to a digital temperature controller, a nitrogen inlet tube connected to a source of either vacuum or dry nitrogen and a mechanical stirrer, was charged with a mixture of 2573 g of Norpar<sup>TM</sup> 12, 828 g of TCHMA, 21 g of EMA, 26.8 g of 98% (w/w) HEMA and 8.75 g of V601. While stirring the mixture, the reaction flask was purged with vacuum at 40 torr for 10 min., followed by nitrogen to break down the vacuum, and was purged with vacuum again at 40 torr for 10 min., followed by nitrogen to break down the vacuum. The nitrogen flow rate was then reduced to approximately 0.5 liters/minute. The mixture was heated to 75° C. for 4 hours. The conversion was quantitative.

25 The mixture was then heated to 100° C. and held at that temperature for 1 hour to destroy any residual V-601, and then was cooled down to 70° C. The nitrogen inlet tube was then removed, and 1.36 g of 95% (w/w) DBTDL were added to the mixture, followed by 41.1 g of TMI. The TMI was pulled slowly into the mixture over the course of approximately 2 minutes while stirring the reaction mixture. The nitrogen inlet tube was replaced and the mixture was allowed to react at 70° C. for 2 hours, at which time the conversion was quantitative.

30 The cooled mixture was a viscous, transparent liquid containing no visible insoluble matter. The percent solids of the liquid mixture was determined to be 25.7% (w/w) using the thermo-gravimetric method described above. Subsequent determination of molecular weight was made using the GPC method described above; the copolymer had a  $M_w$  of 216,500 Da and  $M_w/M_n$  of 2.4 based on two independent measurements. The measured glass transition temperature of the polymer was 123.9° C., as determined by DSC using the method described above. The product was a copolymer of TCHMA, EMA and HEMA containing random side chains of TMI and was designated herein as TCHMA/EMA/HEMA-TMI (94.5/2.5/3-4.7% w/w). It can be used to make an organosol.

#### Example 4

35 Example 4 was prepared similarly to Example 3, except that at the beginning of the reactions, a mixture of 2573 g of Norpar<sup>TM</sup>12, 806 g of TCHMA, 42 g EMA, 26.8 g of 98% (w/w) HEMA, and 8.75g of V-601 was charged to the reactor.

40 The cooled mixture was a viscous, transparent liquid containing no visible insoluble matter. The percent solids of

27

the liquid mixture was determined to be 25.5% (w/w) using the thermo-gravimetric method described above. Subsequent determination of molecular weight was made using the GPC method described above; the copolymer had a  $M_w$  of 218,400 Da and  $M_w/M_n$  of 2.5 based on two independent measurements. The measured glass transition temperature of the polymer was 122.0° C., as determined by DSC using the method described above. The product was a copolymer of TCHMA, EMA and HEMA containing random side chains of TMI and was designated herein as TCHMA/EMA/HEMA-TMI (92/5/3-4.7% w/w). It can be used to make an organosol.

## Example 5

Example 5 was prepared similarly to Example 3, except that at the beginning of the reactions, a mixture of 2573 g of Norpar<sup>TM</sup>12, 785 g of TCHMA, 64 g EMA, 26.8 g of 98% (w/w) HEMA and 8.75g of V-601 was charged to the reactor.

The cooled mixture was a viscous, transparent liquid containing no visible insoluble matter. The percent solids of the liquid mixture was determined to be 25.4% (w/w) using the thermo-gravimetric method described above. Subsequent determination of molecular weight was made using the GPC method described above; the copolymer had a  $M_w$  of 240,400 Da and  $M_w/M_n$  of 2.4 based on two independent measurements. The measured glass transition temperature of the polymer was 119.2° C., as determined by DSC using the method described above. The product was a copolymer of TCHMA, EMA and HEMA containing random side chains of TMI and was designated herein as TCHMA/EMA/HEMA-TMI (89.5/7.5/3-4.7% w/w). It can be used to make an organosol.

## Example 6

Example 6 was prepared similarly to Example 3, except that at the beginning of the reactions, a mixture of 2573 g of Norpar<sup>TM</sup>12, 764 g of TCHMA, 85 g EMA, 26.8 g of 98% (w/w) HEMA and 8.75 g of V-601 was charged to the reactor.

The cooled mixture was a viscous, transparent liquid containing no visible insoluble matter. The percent solids of the liquid mixture was determined to be 25.4% (w/w) using the thermo-gravimetric method described above. Subsequent determination of molecular weight was made using the GPC method described above; the copolymer had a  $M_w$  of 234,100 Da and  $M_w/M_n$  of 2.5 based on two independent measurements. The measured glass transition temperature of the polymer was 104.4° C., as determined by DSC using the method described above. The product was a copolymer of TCHMA, EMA and HEMA containing random side chains of TMI and was designated herein as TCHMA/EMA/HEMA-TMI (87/10/3-4.7% w/w). It can be used to make an organosol.

## Example 7 (Comparative)

Example 7 was prepared similarly to Example 3, except that at the beginning of the reactions, a mixture of 2660 g of Norpar<sup>TM</sup>12, 630 g of TCHMA, 131.25 g EMA, 26.8 g of 98% (w/w) HEMA and 8.75 g of V-601 was charged to the reactor.

The cooled mixture was a viscous, hazy liquid with phase separation. The product was a copolymer of TCHMA, EMA and HEMA containing random side chains of TMI and was designated herein as TCHMA/EMA/HEMA-TMI (82/15/3-

28

4.7% w/w). It is not used to make an organosol due to the phase separation of the polymer in Norpar<sup>TM</sup>12.

## Example 8

A 32 ounce (0.72 liter), narrow-mouthed glass bottle was charged with 478 g of Norpar<sup>TM</sup>12, 149.5 g of TCHMA, 8.1 g of EA, 5.0 g of 98% (w/w) HEMA and 1.6 g of V-601. The bottle was then sealed with a screw cap fitted with a Teflon liner and the cap was secured in place using electrical tape. The sealed bottle was inserted into a metal cage assembly and installed on the agitator assembly of an Atlas Launder-Ometer (Atlas Electric Devices Company, Chicago, Ill.). The Launder-Ometer was operated at its fixed agitation speed of 42 RPM with a water bath temperature of 75° C. The mixture in the sealed bottle was allowed to react for 4 hours at which time the conversion of monomer to polymer was quantitative. The mixture was heated to 100° C. for 1 hour to destroy any residual V-601, and then was cooled to room temperature.

The bottle was then opened and 0.25 g of 95% (w/w) DBTDL and 7.6 g of TMI were added to the mixture. The bottle was sealed again and returned to the Atlas Launder-Ometer as described above. The Launder-Ometer was operated at its fixed agitation speed of 42 RPM with a water bath temperature of 70° C. The mixture was allowed to react for 2 hours, at which time the conversion was quantitative.

The cooled mixture was a viscous, transparent liquid containing no visible insoluble matter. The percent solids of the liquid mixture was determined to be 25.8% (w/w) using the thermo-gravimetric method described above. Subsequent determination of molecular weight was made using the GPC method described above; the copolymer had a  $M_w$  of 221,900 Da and  $M_w/M_n$  of 2.9 based on two independent measurements. The measured glass transition temperature of the polymer was 119.6° C., as determined by DSC using the method described above. The product was a copolymer of TCHMA, EA and HEMA containing random side chains of TMI and was designated herein as TCHMA/EA/HEMA-TMI (92/5/3-4.7% wlw). It can be used to make an organosol.

## Example 9

Example 9 was prepared similarly to Example 8, except that at the beginning of the reactions, a mixture of 478 g of Norpar<sup>TM</sup>12, 141.4 g of TCHMA, 16.2 g of EA, 5.0 g of 98% (w/w) HEMA and 1.63 g of V-601 was charged to the narrow-mouthed glass bottle.

The cooled mixture was a viscous, transparent liquid containing no visible insoluble matter. The percent solids of the liquid mixture was determined to be 25.9% (w/w) using the thermo-gravimetric method described above. Subsequent determination of molecular weight was made using the GPC method described above; the copolymer had a  $M_w$  of 215,650 Da and  $M_w/M_n$  of 2.8 based on two independent measurements. The measured glass transition temperature of the polymer was 105.6° C., as determined by DSC using the method described above. The product was a copolymer of TCHMA, EA and HEMA containing random side chains of TMI and was designated herein as TCHMA/EA/HEMA-TMI (87/10/3-4.7% w/w). It can be used to make an organosol.

Example 10 was prepared similarly to Example 8, except that at the beginning of the reactions, a mixture of 478 g of Norpar<sup>TM</sup>12, 133.2 g of TCHMA, 24.4 g of EA, 5.0 g of 98% (w/w) HEMA and 1.63 g of V-601 was charged to the narrow-mouthed glass bottle.

The cooled mixture was a viscous, transparent liquid containing no visible insoluble matter. The percent solids of the liquid mixture was determined to be 25.8% (w/w) using the thermo-gravimetric method described above. Subsequent determination of molecular weight was made using the GPC method described above; the copolymer had a  $M_w$  of 208,000 Da and  $M_w/M_n$  of 2.6 based on two independent measurements. The measured glass transition temperature of the polymer was 91.4° C., as determined by DSC using the method described above. The product was a copolymer of TCHMA, EA and HEMA containing random side chains of TMI and was designated herein as TCHMA/EA/HEMA-TMI (82/15/3-4.7% w/w). It can be used to make an organosol.

## Example 11 (Comparative)

Example 11 was prepared similarly to Example 8, except that at the beginning of the reactions, a mixture of 478 g of Norpar<sup>TM</sup>12, 125.1 g of TCHMA, 32.5 g of EA, 5.0 g of 98% (w/w) HEMA and 1.63 g of V-601 was charged to the narrow-mouthed glass bottle.

The cooled mixture was a viscous, hazy liquid with phase separation. The product was a copolymer of TCHMA, EA and HEMA containing random side chains of TMI and was designated herein as TCHMA/EA/HEMA-TMI (77/20/3-4.7% w/w). It is not used to make an organosol due to the phase separation of the polymer in Norpar<sup>TM</sup>12.

## Example 12

Example 12 was prepared similarly to Example 8, except that at the beginning of the reactions, a mixture of 478 g of Norpar<sup>TM</sup>12, 108.9 g of LMA, 48.7 g of EMA, 5.0 g of 98% (w/w) HEMA and 1.63 g of V-601 was charged to the narrow-mouthed glass bottle.

The cooled mixture was a viscous, transparent liquid containing no visible insoluble matter. The percent solids of the liquid mixture was determined to be 23.4% (w/w) using the thermo-gravimetric method described above. Subse-

quent determination of molecular weight was made using the GPC method described above; the copolymer had a  $M_w$  of 104,750 Da and  $M_w/M_n$  of 2.2 based on two independent measurements. The measured glass transition temperature of the polymer was -5.3° C., as determined by DSC using the method described above. The product was a copolymer of LMA, EMA and HEMA containing random side chains of TMI and was designated herein as LMA/EMA/HEMA-TMI (67/30/3-4.7% w/w). It can be used to make an organosol.

Example 13 was prepared similarly to Example 8, except that at the beginning of the reactions, a mixture of 478 g of Norpar<sup>TM</sup>12, 92.6 g of LMA, 65.0 g of EMA, 5.0 g of 98% (w/w) HEMA and 1.63 g of V-601 was charged to the narrow-mouthed glass bottle.

The cooled mixture was a viscous, transparent liquid containing no visible insoluble matter. The percent solids of the liquid mixture was determined to be 23.5% (w/w) using the thermo-gravimetric method described above. Subsequent determination of molecular weight was made using the GPC method described above; the copolymer had a  $M_w$  of 102,950 Da and  $M_w/M_n$  of 2.4 based on two independent measurements. The measured glass transition temperature of the polymer was 1.1° C., as determined by DSC using the method described above. The product was a copolymer of LMA, EMA and HEMA containing random side chains of TMI and was designated herein as LMA/HEMA-TMI (57/40/3-4.7% w/w). It can be used to make an organosol.

## Example 14 (Comparative)

Example 14 was prepared similarly to Example 8, except that at the beginning of the reactions, a mixture of 478 g of Norpar<sup>TM</sup>12, 84.5 g of LMA, 73.1 g of EMA, 5.0 g of 98% (w/w) HEMA and 1.63 g of V-601 was charged to the narrow-mouthed glass bottle.

The cooled mixture was a viscous, hazy liquid with phase separation. The product was a copolymer of LMA, EMA and HEMA containing random side chains of TMI and was designated herein as LMA/EMA/HEMA-TMI (52/45/3-4.7% w/w). It is not used to make an organosol due to the phase separation of the polymer in Norpar<sup>TM</sup>12.

The compositions of the graft stabilizers of Example 1 to 14 are summarized in the following Table.

TABLE 2

| Graft Stabilizers Containing Non-Sorptive Segments |                                     |                       |                                     |                       |
|----------------------------------------------------|-------------------------------------|-----------------------|-------------------------------------|-----------------------|
| Examples                                           | Compositions (% (w/w))              | Non-Sorptive Segments | Polymer in Norpar <sup>TM</sup> -12 | T <sub>g</sub> (° C.) |
| 1 Comp.                                            | TCHMA/HEMA-TMI (97/3-4.7)           | None                  | Soluble                             | 123.0                 |
| 2 Comp.                                            | LMA/HEMA-TMI (97/3-4.7)             | None                  | Soluble                             | -63.0                 |
| 3                                                  | TCHMA/EMA/HEMA-TMI (94.5/2.5/3-4.7) | EMA, 2.5%             | Soluble                             | 123.9                 |
| 4                                                  | TCHMA/EMA/HEMA-TM (92/5/3-4.7)      | EMA, 5%               | Soluble                             | 122.0                 |
| 5                                                  | TCHMA/EMA/HEMA-TMI (89.5/7.5/3-4.7) | EMA, 7.5%             | Soluble                             | 119.2                 |
| 6                                                  | TCHMA/EMA/HEMA-TMI (87/10/3-4.7)    | EMA, 10%              | Slightly Phase sep.                 | 104.4                 |
| 7 Comp.                                            | TCHMA/EMA/HEMA-TMI (82/15/3-4.7)    | EMA, 15%              | Phase sep.                          | —                     |
| 8                                                  | TCHMA/EA/HEMA-TMI (92/5/3-4.7)      | EA, 5%                | Soluble                             | 119.6                 |
| 9                                                  | TCHMA/EA/HEMA-TMI (87/10/3-4.7)     | EA, 10%               | Soluble                             | 105.6                 |
| 10                                                 | TCHMA/EA/HEMA-TMI (82/15/3-4.7)     | EA, 15%               | Soluble                             | 91.4                  |
| 11 Comp.                                           | TCHMA/EA/HEMA-TMI (77/20/3-4.7)     | EA, 20%               | Phase sep.                          | —                     |
| 12                                                 | LMA/EMA/HEMA-TMI (67/30/3-4.7)      | EMA, 30%              | Soluble                             | -5.3                  |
| 13                                                 | LMA/EMA/HEMA-TMI (57/40/3-4.7)      | EMA, 40%              | Soluble                             | 1.1                   |
| 14 Comp.                                           | LMA/EMA/HEMA-TMI (52/45/3-4.7)      | EMA, 45%              | Phase sep.                          | —                     |

31

Example 15-25

Preparations of Organosols

Example 15 (Comparative)

This is a comparative example using the graft stabilizer in Example 1 to prepare an organosol with a core/shell (D/S) ratio of 6/1. A 5000 ml open head reactor equipped with a condenser, a thermocouple connected to a digital temperature controller, a nitrogen inlet tube connected to a source of dry nitrogen and a mechanical stirrer with anchor blade, was charged with a mixture of 2899.0 g of Norpar<sup>TM</sup> 12, 360.0 g of EMA, and 237.2 g of the graft stabilizer mixture from Example 1, and 4.2 g of V-601. While stirring the mixture, the reaction flask was purged with dry nitrogen for 30 minutes at flow rate of approximately 2 liters/minute and was then reduced to approximately 0.5 liter/minute. The mixture was heated to 75° C. for 5 hours. The conversion was quantitative.

Approximately 500 g of n-heptane were added to the cooled organosol, and the resulting mixture was stripped of residual monomer using a rotary evaporator equipped with a dry ice/acetone condenser and operating at a temperature of 90° C. and a vacuum of approximately 15 mm Hg. The stripped organosol was cooled to room temperature, yielding an opaque white dispersion.

This organosol was designated TCHMA/HEMA-TMI//EMA (97/3-4.7//100% (w/w)) and can be used to make ink formulations. The percent solids of the organosol dispersion after stripping was determined to be 13.3% (w/w) using the thermo-gravimetric method described above. Subsequent determination of average particles size was made using the laser diffraction method described above; the organosol had a volume average diameter 30.6  $\mu$ m. The measured glass transition temperature of the polymer was 66.7° C., as determined by DSC using the method described above.

Example 16 (Comparative)

This is a comparative example using the graft stabilizer in Example 2 to prepare an organosol with a core/shell (D/S) ratio of 8/1. To a clean 60-gallon reactor, equipped with a condenser, a thermocouple connected to a digital temperature controller, a nitrogen inlet tube connected to a source of dry nitrogen and a mixer, was charged with a mixture of 146.5 lbs of Norpar<sup>TM</sup>12 and 13.4 lbs of the graft stabilizer mixture from Example 2 along with an additional 1 lb of Norpar<sup>TM</sup>12 to rinse the pump. Agitation was then turned on at a rate of 60 RPM, and temperature was checked to ensure maintenance at ambient. Next 0.48 lb of V-64 was added, along with 1 lb of Norpar<sup>TM</sup>12 to rinse the container. Finally 28.4 lbs of EMA was added along with 28.4 lbs Norpar<sup>TM</sup>12 for rinsing the pump. A vacuum was then applied at 16 torr for 10 minutes, and then broken by a nitrogen blanket. A second vacuum was pulled at 22 torr for 10 minutes, and then agitation stopped to verify that no bubbles were coming out of the solution. The vacuum was then broken with a nitrogen blanket and a light flow of nitrogen of 0.5 CFH (cubic foot per hour) was applied. Agitation of 85 RPM was resumed and the temperature of the reactor was heated to 70° C. and maintained for 16 hours. The conversion was quantitative.

The resulting mixture was stripped of residual monomer by adding 40 lbs of n-heptane and agitation was held at 90

32

RPM with the batch heated to 95° C. The nitrogen flow was stopped and a vacuum of 165 torr was pulled and held for 10 minutes. The vacuum was then increased to 105, 66, and 40 torr, being held at each level for 10 minutes. Finally, the vacuum was increased to 26 torr and held for 30 minutes. The vacuum was then broken, and the stripped organosol was cooled to room temperature, yielding an opaque white dispersion.

10 This organosol was designated LMA/HEMA-TMI//EMA (97/3-4.7//100% (w/w)) and can be used to make ink formulations. The percent solids of the organosol dispersion after stripping was determined to be 18.6% (w/w) using the thermo-gravimetric method described above. Subsequent 15 determination of average particles size was made using the laser diffraction method described above; the organosol had a volume average diameter 8.9  $\mu$ m. The measured glass transition temperature of the polymer was 64.3° C., as determined by DSC using the method described above.

Example 17

Example 17 was prepared similarly to Example 15, except that at the beginning of the reactions, a mixture of 2902 g of Norpar<sup>TM</sup>12, 360 g of EMA, 233.5 g of the graft stabilizer mixture from Example 3, and 4.2 g of V-601 were charged to the reactor.

20 This organosol was designated TCHMA/EMA/HEMA-TMI//EMA (94.5/2.5/3-4.7//100% (w/w)) and can be used to make ink formulations. The percent solids of the organosol dispersion after stripping was determined to be 13.1% (w/w) using the thermo-gravimetric method described above. Subsequent 25 determination of average particles size was made using the laser diffraction method described above; the organosol had a volume average diameter 26.7  $\mu$ m. The measured glass transition temperature of the polymer was 65.6° C., as determined by DSC using the method described above.

Example 18

Example 18 was prepared similarly to Example 15, except that at the beginning of the reactions, a mixture of 2901 g of Norpar<sup>TM</sup>12, 360 g of EMA, 235.3 g of the graft stabilizer mixture from Example 4, and 4.2 g of V-601 were charged to the reactor.

30 This organosol was designated TCHMA/EMA/HEMA-TMI//EMA (92/5/3-4.7//100% (w/w)) and can be used to make ink formulations. The percent solids of the organosol dispersion after stripping was determined to be 12.4% (w/w) using the thermo-gravimetric method described above. Subsequent 35 determination of average particles size was made using the laser diffraction method described above; the organosol had a volume average diameter 40.0  $\mu$ m. The measured glass transition temperature of the polymer was 63.4° C., as determined by DSC using the method described above.

Example 19

Example 19 was prepared similarly to Example 15, except that at the beginning of the reactions, a mixture of 2900 g of Norpar<sup>TM</sup>12, 360 g of EMA, 236.2 g of the graft stabilizer mixture from Example 5, and 4.2 g of V-601 were charged to the reactor.

33

This organosol was designated TCHMA/EMA/HEMA-TMI//EMA (89.5/7.5/3-4.7//100% (w/w)) and can be used to make ink formulations. The percent solids of the organosol dispersion after stripping was determined to be 12.0% (w/w) using the thermo-gravimetric method described above. Subsequent determination of average particles size was made using the laser diffraction method described above; the organosol had a volume average diameter 33.1  $\mu\text{m}$ . The measured glass transition temperature of the polymer was 66.2  $^{\circ}\text{C}$ ., as determined by DSC using the method described above.

## Example 20

Example 20 was prepared similarly to Example 15, except that at the beginning of the reactions, a mixture of 2900 g of Norpar<sup>TM</sup>12, 360 g of EMA, 232.6 g of the graft stabilizer mixture from Example 6, and 4.2 g of V-601 were charged to the reactor.

This organosol was designated TCHMA/EMA/HEMA-TMI//EMA (87/10/3-4.7//100% (w/w)) and can be used to make ink formulations. The percent solids of the organosol dispersion after stripping was determined to be 13.0% (w/w) using the thermo-gravimetric method described above. Subsequent determination of average particles size was made using the laser diffraction method described above; the organosol had a volume average diameter 32.8  $\mu\text{m}$ . The measured glass transition temperature of the polymer was 70.4  $^{\circ}\text{C}$ ., as determined by DSC using the method described above.

## Example 21

Example 21 was prepared similarly to Example 15, except that at the beginning of the reactions, a mixture of 2903 g of Norpar<sup>TM</sup>12, 360 g of EMA, 232.6 g of the graft stabilizer mixture from Example 8, and 4.2 g of V-601 were charged to the reactor.

This organosol was designated TCHMA/EA/HEMA-TMI//EMA (92/5/3-4.7//100% (w/w)) and can be used to make ink formulations. The percent solids of the organosol dispersion after stripping was determined to be 11.1% (w/w) using the thermo-gravimetric method described above. Subsequent determination of average particles size was made using the laser diffraction method described above; the organosol had a volume average diameter 38.1  $\mu\text{m}$ . The measured glass transition temperature of the polymer was 68.5  $^{\circ}\text{C}$ ., as determined by DSC using the method described above.

## Example 22

Example 22 was prepared similarly to Example 15, except that at the beginning of the reactions, a mixture of 2904 g of Norpar<sup>TM</sup>12, 360 g of EMA, 231.7 g of the graft stabilizer mixture from Example 9, and 4.2 g of V-601 were charged to the reactor.

This organosol was designated TCHMA/EA/HEMA-TMI//EMA (87/10/3-4.7//100% (w/w)) and can be used to make ink formulations. The percent solids of the organosol dispersion after stripping was determined to be 11.3% (w/w) using the thermo-gravimetric method described above. Sub-

34

sequent determination of average particles size was made using the laser diffraction method described above; the organosol had a volume average diameter 44.5  $\mu\text{m}$ . The measured glass transition temperature of the polymer was 71.5  $^{\circ}\text{C}$ ., as determined by DSC using the method described above.

## Example 23

Example 23 was prepared similarly to Example 15, except that at the beginning of the reactions, a mixture of 2903 g of Norpar<sup>TM</sup>12, 360 g of EMA, 232.6 g of the graft stabilizer mixture from Example 10, and 4.2 g of V-601 were charged to the reactor.

This organosol was designated TCHMA/EA/HEMA-TMI//EMA (82/15/3-4.7//100% (w/w)) and can be used to make ink formulations. The percent solids of the organosol dispersion after stripping was determined to be 12.6% (w/w) using the thermo-gravimetric method described above. Subsequent determination of average particles size was made using the laser diffraction method described above; the organosol had a volume average diameter 44.3  $\mu\text{m}$ . The measured glass transition temperature of the polymer was 71.3  $^{\circ}\text{C}$ ., as determined by DSC using the method described above.

## Example 24

Example 24 was prepared similarly to Example 15, except that at the beginning of the reactions, a mixture of 2879 g of Norpar<sup>TM</sup>12, 360 g of EMA, 256.4 g of the graft stabilizer mixture from Example 12, and 4.2 g of V-601 were charged to the reactor.

This organosol was designated LMA/EMA/HEMA-TMI//EMA (67/30/3-4.7//100% (w/w)) and can be used to make ink formulations. The percent solids of the organosol dispersion after stripping was determined to be 12.3% (w/w) using the thermo-gravimetric method described above. Subsequent determination of average particles size was made using the laser diffraction method described above; the organosol had a volume average diameter 19.6  $\mu\text{m}$ . The measured glass transition temperature of the polymer was 63.7  $^{\circ}\text{C}$ ., as determined by DSC using the method described above.

## Example 25

Example 24 was prepared similarly to Example 15, except that at the beginning of the reactions, a mixture of 2880 g of Norpar<sup>TM</sup>12, 360 g of EMA, 255.3 g of the graft stabilizer mixture from Example 13, and 4.2 g of V-601 were charged to the reactor.

This organosol was designated LMA/EMA/HEMA-TMI//EMA (57/40/3-4.7//100% (w/w)) and can be used to make ink formulations. The percent solids of the organosol dispersion after stripping was determined to be 11.6% (w/w) using the thermo-gravimetric method described above. Subsequent determination of average particles size was made using the laser diffraction method described above; the organosol had a volume average diameter 24.8  $\mu\text{m}$ . The measured glass transition temperature of the polymer was 65.9  $^{\circ}\text{C}$ ., as determined by DSC using the method described above.

The compositions of the organosol copolymers formed in Examples 15 to 25 are summarized in the following table:

TABLE 3

## Organosols Containing Non-Sorptive Segments in the Shells

| Examples | Graft Copolymer Compositions<br>(% w/w)       | T <sub>g</sub><br>(° C.) | Non-Sorptive<br>Segments,<br>(w/w) |
|----------|-----------------------------------------------|--------------------------|------------------------------------|
| 15 Comp. | TCHMA/HEMA-TMI//EMA (97/3-4.7//100)           | 66.7                     | None                               |
| 16 Comp. | LMA/HEMA-TMI//EMA (97/3-4.7//100)             | 64.3                     | None                               |
| 17       | TCHMA/EMA/HEMA-TMI//EMA (94.5/2.5/3-4.7//100) | 65.6                     | EMA, 2.5%                          |
| 18       | TCHMA/EMA/HEMA-TMI//EMA (92/5/3-4.7//100)     | 63.4                     | EMA, 5%                            |
| 19       | TCHMA/EMA/HEMA-TMI//EMA (89.5/7.5/3-4.7//100) | 66.2                     | EMA, 7.5%                          |
| 20       | TCHMA/EMA/HEMA-TMI//EMA (87/10/3-4.7//100)    | 70.4                     | EMA, 10%                           |
| 21       | TCHMA/EA/HEMA-TMI//EMA (92/5/3-4.7//100)      | 68.5                     | EA, 5%                             |
| 22       | TCHMA/EA/HEMA-TMI//EMA (87/10/3-4.7//100)     | 71.5                     | EA, 10%                            |
| 23       | TCHMA/EA/HEMA-TMI//EMA (82/15/3-4.7//100)     | 71.3                     | EA, 15%                            |
| 24       | LMA/EMA/HEMA-TMI//EMA (67/30/3-4.7//100)      | 63.7                     | EMA, 30%                           |
| 25       | LMA/EMA/HEMA-TMI//EMA (57/40/3-4.7//100)      | 65.9                     | EMA, 40%                           |

## Examples 26-47

## Preparation of Liquid Toner Compositions

For characterization of the prepared liquid toner compositions in these Examples, the following properties were measured: percent solids, size-related properties (particle size); charge-related properties (bulk and free phase conductivity, dynamic mobility); and charge/developed reflectance optical density (Z/ROD), a parameter that is directly proportional to the toner charge/mass (Q/M), and fused image erasure resistance.

## Example 26 (Comparative)

This is a comparative example of preparing a cyan liquid toner at an organosol to pigment ratio of 6 using the organosol prepared in example 15. 251.3 g of the organosol from example 15 were combined with 42.1 g of Norpar<sup>TM</sup>12, 5.6 g of Pigment Blue 15:2 (Sun Chemical Company, Cincinnati, Ohio) and 1.0 g of 5.67% (w/w) Zirconium HEX-CEM solution in a 16 ounce glass jar. This mixture was then milled in a 0.5 liter vertical bead mill (Model 6TSG-1/4, Aimex Co., Ltd., Tokyo, Japan) charged with 390 g of 1.3 mm diameter Potters glass beads (Potters Industries, Inc., Parsippany, N.J.). The mill was operated at 2,000 RPM for 20 min. with a water-bath circulating at 80° C. through the heating jacket of the milling chamber. The temperature of the water-bath was then reduced to 45° C. and the mill was operated at 2,000 RPM for an additional 22 min. At the end of the milling, 187.5 g of Norpar<sup>TM</sup>12 was used to rinse out the mill and reduce the solids percentage of the liquid ink.

Measured percent of solids: 7.9% (w/w)

Measured volume mean particle size: 4.2  $\mu$ m

Measured bulk conductivity: 184 picoMhos/cm

Measured percent free phase conductivity: 0.99%

Measured dynamic mobility: 0.522E-10 (m<sup>2</sup>/Vsec)

Measured Q/M: 206  $\mu$ C/g

Print tested reflection optical density (OD): 1.3

Fused image erasure resistances at different fusing temperatures are summarized in Table 4.

## Example 27 (Comparative)

This is a comparative example of preparing a cyan liquid toner. It was prepared and analyzed similarly to example 26, except that 180.2 g of the organosol from example 16 were

combined with 113.2 g of Norpar<sup>TM</sup>12 and the rest of the ingredients that were listed in example 26 when preparing for the cyan ink milling and that after the 20 min. of milling at 80° C., it was milled at 45° C. for an additional 22 min.

Measured percent of solids: 8.2% (w/w)

Measured volume mean particle size: 5.7  $\mu$ m

Measured bulk conductivity: 65 picoMhos/cm

Measured percent free phase conductivity: 3.2%

Measured dynamic mobility: 0.342E-10 (m<sup>2</sup>/Vsec)

Measured Q/M: 106  $\mu$ C/g

Print tested reflection optical density (OD): 1.3

Fused image erasure resistances at different fusing temperatures are summarized in Table 4.

## Example 28

This is an example of preparing a cyan liquid toner. It was prepared and analyzed similarly to example 26, except that 257.1 g of the organosol from example 17 were combined with 36.3 g of Norpar<sup>TM</sup>12 and the rest of the ingredients that were listed in example 26 when preparing for the cyan ink milling and that after the 20 min. of milling at 80° C., it was milled at 45° C. for an additional 22 min.

Measured percent of solids: 8.2% (w/w)

Measured volume mean particle size: 4.9  $\mu$ m

Measured bulk conductivity: 219 picoMhos/cm

Measured percent free phase conductivity: 1.34%

Measured dynamic mobility: 0.831E-10 (m<sup>2</sup>/Vsec)

Measured Q/M: 207  $\mu$ C/g

Print tested reflection optical density (OD): 1.1

Fused image erasure resistances at different fusing temperatures are summarized in Table 4.

## Example 29

This is an example of preparing a cyan liquid toner. It was prepared and analyzed similarly to example 26, except that 269.6 g of the organosol from example 18 were combined with 23.9 g of Norpar<sup>TM</sup>12 and the rest of the ingredients that were listed in example 26 when preparing for the cyan ink milling and that after the 20 min. of milling at 80° C., it was milled at 45° C. for an additional 30 min.

Measured percent of solids: 8.8% (w/w)

Measured volume mean particle size: 4.7  $\mu$ m

Measured bulk conductivity: 215 picoMhos/cm

Measured percent free phase conductivity: 0.27%

Measured dynamic mobility: 0.637E-10 (m<sup>2</sup>/Vsec)

Measured Q/M: 163  $\mu$ C/g

37

Print tested reflection optical density (OD): 1.3  
 Fused image erasure resistances at different fusing temperatures are summarized in Table 4.

## Example 30

This is an example of preparing a cyan liquid toner. It was prepared and analyzed similarly to example 26, except that 278.6 g of the organosol from example 19 was combined with 14.9 g of Norpar<sup>TM</sup>12 and the rest of the ingredients that were listed in example 26 when preparing for the cyan ink milling and that after the 20 min. of milling at 80° C., it was milled at 45° C. for an additional 27 min.

Measured percent of solids: 8.7% (w/w)

Measured volume mean particle size: 5.5  $\mu\text{m}$

Measured bulk conductivity: 243 picoMhos/cm

Measured percent free phase conductivity: 0.46%

Measured dynamic mobility: 0.839E-10 ( $\text{m}^2/\text{Vsec}$ )

Measured Q/M: 189  $\mu\text{C/g}$

Print tested reflection optical density (OD): 1.2

Fused image erasure resistances at different fusing temperatures are summarized in Table 4.

## Example 31

This is an example of preparing a cyan liquid toner. It was prepared and analyzed similarly to example 26, except that 257.1 g of the organosol from example 20 was combined with 36.3 g of Norpar<sup>TM</sup>12 and the rest of the ingredients that were listed in example 26 when preparing for the cyan ink milling and that after the 20 min. of milling at 80° C., it was milled at 45° C. for an additional 13 min.

Measured percent of solids: 8.5% (w/w)

Measured volume mean particle size: 4.9  $\mu\text{m}$

Measured bulk conductivity: 193 picoMhos/cm

Measured percent free phase conductivity: 0.90%

Measured dynamic mobility: 0.646E-10 ( $\text{m}^2/\text{Vsec}$ )

Measured Q/M: 175  $\mu\text{C/g}$

Print tested reflection optical density (OD): 1.3

Fused image erasure resistances at different fusing temperatures are summarized in Table 4.

## Example 32

This is an example of preparing a cyan liquid toner. It was prepared and analyzed similarly to example 26, except that 290.7 g of the organosol from example 21 were combined with 2.8 g of Norpar<sup>TM</sup>12 and the rest of the ingredients that were listed in example 26 when preparing for the cyan ink milling and that after the 20 min. of milling at 80° C., it was milled at 45° C. for an additional 65 min.

Measured percent of solids: 8.3% (w/w)

Measured volume mean particle size: 4.0  $\mu\text{m}$

Measured bulk conductivity: 216 picoMhos/cm

Measured percent free phase conductivity: 0.95%

Measured dynamic mobility: 0.627E-10 ( $\text{m}^2/\text{Vsec}$ )

Measured Q/M: 151  $\mu\text{C/g}$

Print tested reflection optical density (OD): 1.3

Fused image erasure resistances at different fusing temperatures are summarized in Table 4.

## Example 33

This is an example of preparing a cyan liquid toner. It was prepared and analyzed similarly to example 26, except that 295.8 g of the organosol from example 22 were combined with 0.0 g of Norpar<sup>TM</sup>12 and the rest of the ingredients that

38

were listed in example 26 when preparing for the cyan ink milling and that after the 20 min. of milling at 80° C., it was milled at 45° C. for an additional 70 min.

Measured percent of solids: 7.9% (w/w)

Measured volume mean particle size: 4.1  $\mu\text{m}$

Measured bulk conductivity: 174 picoMhos/cm

Measured percent free phase conductivity: 0.93%

Measured dynamic mobility: 0.559E-10 ( $\text{m}^2/\text{Vsec}$ )

Measured Q/M: 145  $\mu\text{C/g}$

Print tested reflection optical density (OD): 1.3

Fused image erasure resistances at different fusing temperatures are summarized in Table 4.

## Example 34

This is an example of preparing a cyan liquid toner. It was prepared and analyzed similarly to example 26, except that 265.3 g of the organosol from example 23 were combined with 28.1 g of Norpar<sup>TM</sup>12 and the rest of the ingredients that were listed in example 26 when preparing for the cyan ink milling and that after the 20 min. of milling at 80° C., it was milled at 45° C. for an additional 70 min.

Measured percent of solids: 8.3% (w/w)

Measured volume mean particle size: 4.4  $\mu\text{m}$

Measured bulk conductivity: 191 picoMhos/cm

Measured percent free phase conductivity: 1.07%

Measured dynamic mobility: 0.647E-10 ( $\text{m}^2/\text{Vsec}$ )

Measured Q/M: 138  $\mu\text{C/g}$

Print tested reflection optical density (OD): 1.3

Fused image erasure resistances at different fusing temperatures are summarized in Table 4.

## Example 35

This is an example of preparing a cyan liquid toner. It was prepared and analyzed similarly to example 26, except that 271.8 g of the organosol from example 24 were combined with 21.7 g of Norpar<sup>TM</sup>12 and the rest of the ingredients that were listed in example 26 when preparing for the cyan ink milling and that after the 20 min. of milling at 80° C., it was milled at 45° C. for an additional 100 min.

Measured percent of solids: 8.2% (w/w)

Measured volume mean particle size: 4.2  $\mu\text{m}$

Measured bulk conductivity: 264 picoMhos/cm

Measured percent free phase conductivity: 2.09%

Measured dynamic mobility: 0.709E-10 ( $\text{m}^2/\text{Vsec}$ )

Measured Q/M: 167  $\mu\text{C/g}$

Print tested reflection optical density (OD): 1.4

Fused image erasure resistances at different fusing temperatures are summarized in Table 4.

## Example 36

This is an example of preparing a cyan liquid toner. It was prepared and analyzed similarly to example 26, except that 288.2 g of the organosol from example 25 were combined with 5.3 g of Norpar<sup>TM</sup>12 and the rest of the ingredients that were listed in example 26 when preparing for the cyan ink milling and that after the 20 min. of milling at 80° C., it was milled at 45° C. for an additional 110 min.

Measured percent of solids: 8.4% (w/w)

Measured volume mean particle size: 4.6  $\mu\text{m}$

Measured bulk conductivity: 246 picoMhos/cm

Measured percent free phase conductivity: 2.32%

Measured dynamic mobility: 0.769E-10 ( $\text{m}^2/\text{Vsec}$ )

Measured Q/M: 158  $\mu\text{C/g}$

Print tested reflection optical density (OD): 1.4

39

Fused image erasure resistances at different fusing temperatures are summarized in Table 4.

## Example 37

This is a comparative example of preparing a magenta liquid toner. It was prepared and analyzed similarly to example 26, except that 244.4 g of the organosol from example 15 were combined with 48.0 g of Norpar<sup>TM</sup>12, 3.9 g of Pigment Red 146 (available from Dianippon Ink and Chemical, Inc., Tokyo, Japan as FR4580), 1.3 g Pigment Red 81:4 (Magruder Color Company, Inc., Elizabeth, N.J.), 1.3 g of Pigment Red 269 (Magruder Color Company, Inc., Elizabeth, N.J.), and 1.1 g of 5.67% (w/w) Zirconium HEX-CEM solution. After 30 min. of milling at 55° C., the liquid toner was milled at 45° C. for an additional 5 min.

Measured percent of solids: 7.5% (w/w)  
 Measured volume mean particle size: 5.3  $\mu$ m  
 Measured bulk conductivity: 97 picoMhos/cm  
 Measured percent free phase conductivity: 0.95%  
 Measured dynamic mobility: 0.331 E-10 (m<sup>2</sup>/Vsec)  
 Measured Q/M: 119  $\mu$ C/g  
 Print tested reflection optical density (OD): 1.1  
 Fused image erasure resistances at different fusing temperatures are summarized in Table 4.

## Example 38

This is a comparative example of preparing a magenta liquid toner. It was prepared and analyzed similarly to example 37, except that 175.2 g of the organosol from example 16 were combined with 117.2 g of Norpar<sup>TM</sup>12, and the rest of the ingredients that were listed in example 37 when preparing for the magenta ink milling and that after 30 min. of milling at 55° C., it was milled at 45° C. for an additional 5 min.

Measured percent of solids: 8.0% (w/w)  
 Measured volume mean particle size: 6.1  $\mu$ m  
 Measured bulk conductivity: 54 picoMhos/cm  
 Measured percent free phase conductivity: 2.20%  
 Measured dynamic mobility: 0.223E-10 (m<sup>2</sup>/Vsec)  
 Measured Q/M: 88  $\mu$ C/g  
 Print tested reflection optical density (OD): 1.0  
 Fused image erasure resistances at different fusing temperatures are summarized in Table 4.

## Example 39

This is an example of preparing a magenta liquid toner. It was prepared and analyzed similarly to example 37, except that 248.1 g of the organosol from example 17 was combined with 44.3 g of Norpar<sup>TM</sup>12, and the rest of the ingredients that were listed in example 37 when preparing for the magenta ink milling and that after 30 min. of milling at 55° C., it was milled at 45° C. for an additional 5 min.

Measured percent of solids: 8.1% (w/w)  
 Measured volume mean particle size: 4.6  $\mu$ m  
 Measured bulk conductivity: 157 picoMhos/cm  
 Measured percent free phase conductivity: 0.78%  
 Measured dynamic mobility: 0.612E-10 (m<sup>2</sup>/Vsec)  
 Measured Q/M: 131  $\mu$ C/g  
 Print tested reflection optical density (OD): 1.3  
 Fused image erasure resistances at different fusing temperatures are summarized in Table 4.

40

## Example 40

This is an example of preparing a magenta liquid toner. It was prepared and analyzed similarly to example 37, except that 262.1 g of the organosol from example 18 were combined with 30.3 g of Norpar<sup>TM</sup>12, and the rest of the ingredients that were listed in example 37 when preparing for the magenta ink milling and that after 30 min. of milling at 55° C., it was milled at 45° C. for an additional 30 min.

Measured percent of solids: 8.8% (w/w)  
 Measured volume mean particle size: 4.1  $\mu$ m  
 Measured bulk conductivity: 50 picoMhos/cm  
 Measured percent free phase conductivity: 1.10%  
 Measured dynamic mobility: 0.203E-10 (m<sup>2</sup>/Vsec)  
 Measured Q/M: 58  $\mu$ C/g  
 Print tested reflection optical density (OD): 1.1  
 Fused image erasure resistances at different fusing temperatures are summarized in Table 4.

20

## Example 41

This is an example of preparing a magenta liquid toner. It was prepared and analyzed similarly to example 37, except that 270.8 g of the organosol from example 19 was combined with 21.5 g of Norpar<sup>TM</sup>12, and the rest of the ingredients that were listed in example 37 when preparing for the magenta ink milling and that after 30 min. of milling at 55° C., it was milled at 45° C. for an additional 5 min.

Measured percent of solids: 8.5% (w/w)  
 Measured volume mean particle size: 4.6  $\mu$ m  
 Measured bulk conductivity: 157 picoMhos/cm  
 Measured percent free phase conductivity: 0.82%  
 Measured dynamic mobility: 0.661E-10 (m<sup>2</sup>/Vsec)  
 Measured Q/M: 127  $\mu$ C/g  
 Print tested reflection optical density (OD): 1.3  
 Fused image erasure resistances at different fusing temperatures are summarized in Table 4.

30

## Example 42

This is an example of preparing a magenta liquid toner. It was prepared and analyzed similarly to example 37, except that 250.0 g of the organosol from example 20 were combined with 42.4 g of Norpar<sup>TM</sup>12, and the rest of the ingredients that were listed in example 37 when preparing for the magenta ink milling and that after 30 min. of milling at 55° C., it was milled at 45° C. for an additional 15 min.

Measured percent of solids: 8.4% (w/w)  
 Measured volume mean particle size: 4.1  $\mu$ m  
 Measured bulk conductivity: 61 picoMhos/cm  
 Measured percent free phase conductivity: 0.64%  
 Measured dynamic mobility: 0.264E-10 (m<sup>2</sup>/Vsec)  
 Measured Q/M: 63  $\mu$ C/g  
 Print tested reflection optical density (OD): 1.1  
 Fused image erasure resistances at different fusing temperatures are summarized in Table 4.

40

## Example 43

This is an example of preparing a magenta liquid toner. It was prepared and analyzed similarly to example 37, except that 283.6 g of the organosol from example 21 were combined with 9.7 g of Norpar<sup>TM</sup>12, and the rest of the ingredients that were listed in example 37 when preparing for the



TABLE 4-continued

| Examples<br>Cyan & | <u>Fused Image Erasure Resistance at Different Fusing Temperatures</u> |                  |                                                                    |         |         |         |         |         |         |         |         |         |         |         |
|--------------------|------------------------------------------------------------------------|------------------|--------------------------------------------------------------------|---------|---------|---------|---------|---------|---------|---------|---------|---------|---------|---------|
|                    | $T_g$<br>(° C.)                                                        | Non-<br>Sorptive | Fused Image Erasure Resistance at Different Fusing Temperatures, % |         |         |         |         |         |         |         |         |         |         |         |
| Magenta            | GS                                                                     | CP               | Segments                                                           | 100° C. | 110° C. | 120° C. | 130° C. | 140° C. | 150° C. | 160° C. | 170° C. | 180° C. | 190° C. | 200° C. |
| 33                 | 105.6                                                                  | 71.5             | EA, 10%                                                            | 42.4%   | 72.9%   | 82.7%   | 88.0%   | 89.6%   | 93.1%   | 98.0%   | 99.1%   | 99.2%   | 98.7%   | 98.8%   |
| 44                 | 91.4                                                                   | 71.3             | EA, 15%                                                            | 41.8%   | 50.5%   | 63.0%   | 81.3%   | 76.4%   | 89.3%   | 93.1%   | 97.0%   | 97.5%   | 96.7%   | 95.8%   |
| 34                 | -                                                                      | -                | -                                                                  | -       | -       | -       | -       | -       | -       | -       | -       | -       | -       | -       |
| 45                 | -                                                                      | -                | -                                                                  | -       | -       | -       | -       | -       | -       | -       | -       | -       | -       | -       |
| 35                 | -5.3                                                                   | 63.7             | EMA, 30%                                                           | 60.1%   | 70.2%   | 82.5%   | 88.0%   | 95.5%   | 98.7%   | 98.1%   | 98.7%   | 99.5%   | 99.7%   | 99.2%   |
| 46                 | -                                                                      | -                | -                                                                  | -       | -       | -       | -       | -       | -       | -       | -       | -       | -       | -       |
| 36                 | 1.1                                                                    | 65.9             | EMA, 40%                                                           | 55.2%   | 71.1%   | 89.9%   | 91.7%   | 92.9%   | 97.4%   | 98.4%   | 98.2%   | 99.1%   | 99.0%   | 98.8%   |
| 47                 | -                                                                      | -                | -                                                                  | -       | -       | -       | -       | -       | -       | -       | -       | -       | -       | -       |

GS = Graft Stabilizer

CP = Copolymer

FIG. 1 is a graph showing the fused image erasure resistance of imaged toner compositions plotted against the fusing temperatures of the toner compositions. The text boxes in the graphs of all of the Figures provide S material portion composition information for ease of reference. This Figure demonstrates that the toner compositions of Examples 28 and 39, 29 and 40, 30 and 41 and 31 and 42 (having S material portions comprising soluble component TCHMA in combination with the indicated amount of insoluble component EMA) exhibit superior fused image erasure resistance when fused at certain low fusing temperatures as compared to Comparative Examples 26 and 37 (having S material portions comprising only the soluble component TCHMA).

FIG. 2 is a graph showing the fused image erasure resistance of imaged toner compositions plotted against the fusing temperatures of the toner compositions. This Figure demonstrates that the toner compositions of Examples 26 and 37, 32 and 43, 33 and 44 and 34 and 45 (having S material portions comprising soluble component TCHMA in combination with the indicated amount of insoluble component EA) exhibit superior fused image erasure resistance when fused at certain low fusing temperatures as compared to Comparative Examples 26 and 37 (having S material portions comprising only the soluble component TCHMA).

FIG. 3 is a graph showing the fused image erasure resistance of imaged toner compositions plotted against the fusing temperatures of the toner compositions. This Figure demonstrates that the toner compositions of Examples 35 and 46, and 36 and 47 (having S material portions comprising soluble component LMA in combination with the indicated amount of insoluble component EA) exhibit superior fused image erasure resistance when fused at certain low fusing temperatures as compared to Comparative Examples 27 and 38 (having S material portions comprising only the soluble component LMA).

Other embodiments of this invention will be apparent to those skilled in the art upon consideration of this specification or from practice of the invention disclosed herein. All patents, patent documents, and publications cited herein are incorporated by reference as if individually incorporated. Various omissions, modifications, and changes to the principles and embodiments described herein can be made by one skilled in the art without departing from the true scope and spirit of the invention which is indicated by the following claims.

What is claimed is:

1. A liquid electrographic toner composition comprising:  
a) a liquid carrier having a Kauri-Butanol number less than about 30 mL;
- b) a plurality of toner particles dispersed in the liquid carrier, wherein the toner particles comprise polymeric binder comprising at least one amphiphilic copolymer comprising one or more S material portions and one or more D material portions; and  
wherein the S material portion comprises at least one soluble component and at least one insoluble component, wherein the insoluble component is a reaction product of monomers having an absolute difference in Hildebrand solubility parameter from the liquid carrier of about  $3.0 \text{ MPa}^{1/2}$  or greater.
2. The liquid electrographic toner composition of claim 1, wherein the insoluble component is the reaction product of monomers having an absolute difference in Hildebrand solubility parameter from the liquid carrier of about  $3.15 \text{ MPa}^{1/2}$  or greater.
3. The liquid electrographic toner composition of claim 1, wherein the insoluble component is the reaction product of monomers having an absolute difference in Hildebrand solubility parameter from the liquid carrier of about  $3.30 \text{ MPa}^{1/2}$  or greater.
4. The liquid electrographic toner composition of claim 1, wherein the insoluble component is the reaction product of monomers having an absolute difference in Hildebrand solubility parameter from the liquid carrier of about  $3.40 \text{ MPa}^{1/2}$  or greater.
5. The liquid electrographic toner composition of claim 1, wherein the insoluble component is present in an amount of from about 1% to about 40% of the S material portion.
6. The liquid electrographic toner composition of claim 1, wherein the insoluble component is present in an amount of from about 1% to about 20% of the S material portion.
7. The liquid electrographic toner composition of claim 1, wherein the insoluble component is present in an amount of from about 1% to about 5% of the S material portion.
8. The liquid electrographic toner composition of claim 1, wherein the absolute difference in Hildebrand solubility parameters between the S material portion(s) and the liquid carrier is from about 2 to about  $3.0 \text{ MPa}^{1/2}$ .
9. The liquid electrographic toner composition of claim 1, wherein the insoluble component is randomly arranged within the S material portion of the amphiphilic copolymer.

**45**

10. The liquid electrographic toner composition of claim 1, wherein the insoluble component is prepared by incorporation of a single type of monomer that exhibits the desired solubility parameter as the insoluble component of the S material portion of the amphipathic copolymer.

11. The liquid electrographic toner composition of claim 1, wherein the insoluble component is prepared by incorporation a plurality of monomers, each of which exhibits the desired solubility parameter as the insoluble component of the S material portion of the amphipathic copolymer.

12. The liquid electrographic toner composition of claim 1, wherein the average  $T_g$  of the insoluble component is lower than the average  $T_g$  of the soluble components of the S material portion.

13. The liquid electrographic toner composition of claim 1, wherein the average  $T_g$  of the insoluble component is less than about 70° C., and the average  $T_g$  of the soluble components of the S material portion is greater than about 90° C.

14. The liquid electrographic toner composition of claim 1, wherein the insoluble component has an average  $T_g$  of less than about 0° C., and is from about 1 to about 15% by weight of the S material portion and the soluble component has an average  $T_g$  of greater than about 90° C., and is from about 85 to about 99% by weight of the S material portion.

15. The liquid electrographic toner composition of claim 1, wherein the average  $T_g$  of the insoluble component is higher than the average  $T_g$  of the soluble components of the S material portion.

16. The liquid electrographic toner composition of claim 1, wherein the average  $T_g$  of the insoluble component is greater than about 50° C., and the average  $T_g$  of the soluble components of the S material portion is less than about 0° C.

17. The liquid electrographic toner composition of claim 1, wherein the insoluble component has an average  $T_g$  of is

**46**

greater than about 50° C., and is from about 1 to about 50% by weight of the S material portion; the soluble component has an average  $T_g$  of less than about 0° C., and is from about 50 to about 99% by weight of the S material portion.

18. The liquid electrographic toner composition of claim 1, wherein S material portion comprises the reaction products of soluble monomers selected from the group consisting of trimethyl cyclohexyl methacrylate; t-butyl methacrylate; n-butyl methacrylate; isobornyl(meth)acrylate; 1,6-Hexanediol di(meth)acrylate; 2-hydroxyethyl methacrylate; lauryl methacrylate; and combinations thereof; and further comprises insoluble components that are the reaction products of monomers selected from the group consisting of ethyl acrylate and ethyl methacrylate.

19. A process of preparing a liquid toner composition, comprising

a) preparing toner particles comprise polymeric binder comprising at least one amphipathic copolymer comprising one or more S material portions and one or more D material portions in a preparation liquid carrier wherein the S material portion comprises at least one soluble component and at least one insoluble component, wherein the insoluble component is the reaction product of monomers having an absolute difference in Hildebrand solubility parameter from the preparation liquid carrier of about 3.0 MPa<sup>1/2</sup> or greater;

b) providing said toner particles as a dispersion in a composition liquid carrier having a Kauri-Butanol number less than about 30 mL, wherein the preparation liquid carrier may be the same as or different from the composition liquid carrier.

\* \* \* \* \*